



US010233403B2

(12) **United States Patent**  
**Patil et al.**

(10) **Patent No.:** **US 10,233,403 B2**  
(b4) **Date of Patent:** **Mar. 19, 2019**

(54) **HIGH VISCOSITY INDEX MONOMETHYL ESTER LUBRICATING OIL BASE STOCKS AND METHODS OF MAKING AND USE THEREOF**

(71) Applicant: **ExxonMobil Research and Engineering Company**, Annandale, NJ (US)

(72) Inventors: **Abhimanyu O. Patil**, Westfield, NJ (US); **Satish Bodige**, Wayne, NJ (US); **Stephen Zushma**, Clinton, NJ (US); **Kyle G. Lewis**, Houston, TX (US); **Mark P. Hagemeister**, Mullica Hill, NJ (US)

(73) Assignee: **EXXONMOBiL RESEARCH AND ENGINEERENG COMPANY**, Annandale, NJ (US)

(\*) Notice: Subject to any disclaimer, the term of this patent is extended or adjusted under 35 U.S.C. 154(b) by 112 days.

(21) Appl. No.: **15/384,443**

(22) Filed: **Dec. 20, 2016**

(65) **Prior Publication Data**

US 2018/0119045 A1 May 3, 2018

**Related U.S. Application Data**

(60) Provisional application No. 62/416,966, filed on Nov. 3, 2016.

(51) **Int. Cl.**

**C10M 129/70** (2006.01)  
**C10M 105/34** (2006.01)

(52) **U.S. Cl.**

CPC ..... **C10M 129/70** (2013.01); **C10M 105/34** (2013.01); **C10M 2203/024** (2013.01); **C10M 2203/1006** (2013.01); **C10M 2203/1025** (2013.01); **C10M 2205/0285** (2013.01); **C10M 2205/173** (2013.01); **C10M 2207/281** (2013.01); **C10M 2207/2815** (2013.01); **C10M 2207/2845** (2013.01); **C10N 2220/022** (2013.01); **C10N 2220/028** (2013.01); **C10N 2230/02** (2013.01); **C10N 2230/04** (2013.01); **C10N 2230/10** (2013.01); **C10N 2230/70** (2013.01); **C10N 2230/74** (2013.01); **C10N 2240/04** (2013.01); **C10N 2240/10** (2013.01)

(58) **Field of Classification Search**

CPC ..... C10M 129/70; C10M 2207/281; C10M 2203/024; C10N 2240/04; C10N 2230/02; C10N 2240/10; C10N 2230/74

See application file for complete search history.

(56) **References Cited**

U.S. PATENT DOCUMENTS

|             |        |                  |
|-------------|--------|------------------|
| 2,417,281 A | 3/1947 | Wasson et al.    |
| 2,757,139 A | 7/1956 | Matuszak et al.  |
| 2,870,195 A | 1/1959 | Heininger et al. |

|             |         |                   |
|-------------|---------|-------------------|
| 2,936,856 A | 5/1960  | Braunwarth et al. |
| 2,936,866 A | 5/1960  | Kelly             |
| 3,036,003 A | 5/1962  | Verdol            |
| 3,172,892 A | 3/1965  | Le Suer et al.    |
| 3,210,280 A | 10/1965 | Rich, Jr.         |
| 3,219,666 A | 11/1965 | Norman et al.     |
| 3,316,177 A | 4/1967  | Dorer, Jr.        |
| 3,345,327 A | 10/1967 | Dexter et al.     |
| 3,595,791 A | 7/1971  | Cohen             |
| 3,984,460 A | 10/1976 | Spivack           |
| 4,234,435 A | 11/1980 | Meinhardt et al.  |
| 4,827,064 A | 5/1989  | Wu                |
| 4,827,073 A | 5/1989  | Wu                |

(Continued)

FOREIGN PATENT DOCUMENTS

|    |            |         |
|----|------------|---------|
| DE | 3521711 A1 | 12/1986 |
| EP | 1040115 B1 | 6/2004  |

(Continued)

OTHER PUBLICATIONS

Eastwood, J, "Esters The most Versatile of Base Stock Technologies", Lube-Tech, Lube Magazine, No. 129, Oct. 2015.

Baek, Seung-Yeob, et al. "Synthesis of Succinic Acid Alkyl Half-Ester Derivatives with Improved Lubricity Characteristics", Industrial & Engineering Chemistry Research, ACS Publications, American Chemical Society, vol. 51, No. 9, 2012.

Tabenkin B. et al. "Evaluation of Esters of phenylacetic Acid as Precursors of Penicillin G", Archives of Biochemistry, Academic press, US, vol. 38, Jan. 1952.

The International Search Report and Written Opinion of PCT/US2016/067962 dated Jul. 28, 2017.

The International Search Report and Written Opinion of PCT/US2016/067964 dated May 9, 2017.

(Continued)

*Primary Examiner* — Taiwo Oladapo

(74) *Attorney, Agent, or Firm* — Robert A. Migliorini

(57) **ABSTRACT**

A composition including one or more monomethyl ester compounds represented by the formula:



$\text{R}_1$  is a monomethyl branched  $\text{C}_{15}$  to  $\text{C}_{19}$  alkyl group and  $\text{R}_2$  is an unsubstituted  $\text{C}_2$  to  $\text{C}_{30}$  linear alkyl group. The composition has a viscosity ( $\text{Kv}_{100}$ ) from 1 cSt to 10 cSt at 100° C. as determined by ASTM D445, a viscosity index (VI) from -100 to 300 as determined by ASTM D2270, a pour point from 0° C. to -50° C. as determined by ASTM D97, and a Noack volatility of no greater than 50 percent as determined by ASTM D5800. A process for producing the composition, a lubricating oil base stock and lubricating oil containing the composition, and a method for improving one or more of cold flow properties, thermal and oxidative stability, solubility and dispersancy of polar additives, deposit control and traction control in a lubricating oil by using as the lubricating oil a formulated oil containing the composition.

(56)

## References Cited

| U.S. PATENT DOCUMENTS |         |                                 |
|-----------------------|---------|---------------------------------|
| 4,889,647 A           | 12/1989 | Rowan et al.                    |
| 4,956,122 A           | 9/1990  | Watts et al.                    |
| 4,976,464 A           | 12/1990 | Coyle et al.                    |
| 5,273,672 A           | 12/1993 | Dasai et al.                    |
| 5,488,121 A           | 1/1996  | O'Lenick, Jr.                   |
| 5,639,791 A           | 6/1997  | O'Lenick, Jr.                   |
| 5,705,458 A           | 1/1998  | Roby et al.                     |
| 5,759,968 A           | 6/1998  | Furutani et al.                 |
| 6,008,167 A           | 12/1999 | Appleman et al.                 |
| 6,034,039 A           | 3/2000  | Gomes et al.                    |
| 6,346,504 B1          | 2/2002  | Appelman et al.                 |
| 7,008,909 B2          | 3/2006  | Burgo et al.                    |
| 8,343,899 B2          | 1/2013  | Ichisaka et al.                 |
| 8,673,831 B2          | 3/2014  | Kitching et al.                 |
| 2004/0072703 A1       | 4/2004  | Burgo et al.                    |
| 2005/0014961 A1*      | 1/2005  | Walele ..... A61K 8/37<br>554/1 |
| 2005/0048091 A1       | 3/2005  | Raney et al.                    |
| 2005/0059563 A1       | 3/2005  | Sullivan et al.                 |
| 2007/0172437 A1       | 7/2007  | Bertz et al.                    |
| 2009/0036333 A1       | 2/2009  | Scholier et al.                 |
| 2010/0261628 A1       | 10/2010 | Scherer et al.                  |
| 2011/0039740 A1       | 2/2011  | Kitching et al.                 |
| 2013/0090273 A1       | 4/2013  | Martin et al.                   |
| 2013/0090276 A1       | 4/2013  | Jung et al.                     |
| 2013/0096042 A1       | 4/2013  | Oda                             |
| 2014/0121143 A1       | 5/2014  | Patil et al.                    |
| 2015/0166912 A1       | 6/2015  | Sharko et al.                   |

## FOREIGN PATENT DOCUMENTS

|    |               |         |
|----|---------------|---------|
| EP | 2157159 A1    | 2/2010  |
| EP | 2302022 A1    | 3/2011  |
| GB | 1059296 A     | 12/1967 |
| GB | 1099716 A     | 1/1968  |
| JP | 63066293      | 3/1988  |
| JP | 5159159 B2    | 11/2008 |
| JP | 5334421 B2    | 11/2013 |
| JP | 5334425 B2    | 11/2013 |
| JP | 2014139306 A  | 7/2014  |
| WO | 99/31113 A1   | 6/1999  |
| WO | 200157099 A1  | 8/2001  |
| WO | 2008061709 A1 | 5/2008  |
| WO | 2009130445 A1 | 10/2009 |
| WO | 2003095407 A2 | 11/2011 |
| WO | 2015040937 A1 | 3/2015  |

## OTHER PUBLICATIONS

The International Search Report and Written Opinion of PCT/US2016/067975 dated Jul. 28, 2017.

The International Search Report and Written Opinion of PCT/US2016/067986 dated May 3, 2017.

U.S. Appl. No. 15/384,421.

U.S. Appl. No. 15/384,471.

U.S. Appl. No. 15/384,396.

\* cited by examiner

## 1

**HIGH VISCOSITY INDEX MONOMETHYL  
ESTER LUBRICATING OIL BASE STOCKS  
AND METHODS OF MAKING AND USE  
THEREOF**

**CROSS-REFERENCE TO RELATED  
APPLICATIONS**

This application claims priority to U.S. Provisional Application Ser. No. 62/416,966 filed Nov. 3, 2016, which is herein incorporated by reference in its entirety. This application is related to three (3) other co-pending U.S. applications, filed on even date herewith, and identified by the following titles: Ser. No. 15/384,471 entitled "Low Viscosity Low Volatility Lubricating Oil Base Stocks and Methods of Use Thereof"; Ser. No. 15/384,396 entitled "Low Viscosity Low Volatility Lubricating Oil Base Stocks and Methods of Use Thereof" and Ser. No. 15/384,421 entitled "Low Viscosity Low Volatility Lubricating Oil Base Stocks and Methods of Use Thereof", which are all incorporated herein by reference in their entirety.

**FIELD**

This disclosure relates to high viscosity index, low viscosity, low volatility compositions that include one or more monomethyl ester base stocks of monomethyl branched alcohols and linear aliphatic acids, a process for producing the compositions, a lubricating oil base stock and lubricating oil containing the composition, and a method for improving one or more of thermal and oxidative stability, low temperature properties, solubility and dispersancy of polar additives, deposit control and traction control in a lubricating oil by using as the lubricating oil a formulated oil containing the composition.

**BACKGROUND**

Lubricants in commercial use today are prepared from a variety of natural and synthetic base stocks admixed with various additive packages and solvents depending upon their intended application. The base stocks typically include mineral oils, polyalphaolefins (PAO), gas-to-liquid base oils (GTL), silicone oils, phosphate esters, diesters, polyol esters, and the like.

A major trend for passenger car engine oils (PCEOs) is an overall improvement in quality as higher quality base stocks become more readily available. Typically the highest quality PCEO products are formulated with base stocks such as PAOs or GTL stocks admixed with various additive packages.

For improving fuel economy, base oil viscosity is very important. Substantial improved fuel economy (>2%) requires breakthrough in: (1) base oil volatility (2) durability and (3) friction. Friction losses occur between the moving components within the engine. Models developed to date indicate that fuel economy is heavily influenced by the lubricant properties at high shear. The base stock contributes a greater proportion of the total viscosity under high shear conditions than under low shear. Lowering base stock viscosity is likely to have the largest impact on future fuel economy gains.

Current commercial PAO fluids (e.g., SpectraSyn™ 2) based on hydrocarbon and commercial esters (e.g., 2-ethylhexyl adipate, di-2-ethylhexyl azelate, Esterex™ A32. Esterex™ A34) do not adequately allow formulation of ultra-low viscosity lubricant while still meeting API speci-

## 2

fication (e.g., Noack volatility of 15% or less). In order to formulate ultra-low viscosity lubricant for fuel economy benefit, it is desirable to have low viscosity and low volatility properties co-exist in the same base stock, for meeting volatility requirement. In addition, the base stock should also possess adequate thermal and oxidative stability at high temperature to prevent or minimize deposit formation. Good compatibility with additives commonly used in lubricant formulations (PVL—Passenger Vehicle Lubricants, CVL—Commercial Vehicle Lubricants, industrial lubricants), good low temperature properties, and acceptable viscosity indices are also necessary for the base stocks.

Poly- $\alpha$ -olefins (PAOs) are important lube base stocks with many excellent lubricant properties, including high viscosity index (VI), low volatility and are available in various viscosity range (K<sub>V</sub><sub>100</sub> 2-300 cSt). However, PAOs are paraffinic hydrocarbons with low polarity. This low polarity leads to low solubility and dispersancy for polar additives or sludge generated during service. To compensate for this low polarity, lube formulators usually add one or multiple polar cobase stocks. Ester or alkylated naphthalene (AN) is usually present at 1 wt. % to 50 wt. % levels in many finished lubricant formulations to increase the fluid polarity which improves the solubility of polar additives and sludge.

Therefore, there is a need for polar cobase fluids that provide appropriate solubility and dispersibility for polar additives or sludge generated during service of lubricating oils.

Future automotive and industrial trend suggest that there will be a need for advanced additive technology and synthetic base stocks with substantially better thermal and oxidative stability. This is primarily because of smaller sump sizes that will have more thermal and oxidative stresses on the lubricants. Performance requirements have become more stringent in the past 10 to 20 years and the demand for longer drain intervals has grown steadily. Also, the use of Group II, III and IV base oils is becoming more widespread. Such base oils have very little sulfur content since natural sulfur-containing antioxidants are either absent or removed during the severe refining process.

It is known that lubricant oils used in internal combustion engines and transmission of automobile engines or trucks are subjected to demanding environments during use. These environments result in the lubricant suffering oxidation catalyzed by the presence of impurities in the oil, such as iron (wear) compounds and elevated temperatures. The oxidation manifests itself by increase in acid or viscosity and deposit formation or any combination of these symptoms. These are controlled to some extent by the use of antioxidants which can extend the useful life of the lubricating oil, particularly by reducing or preventing unacceptable viscosity increases. Besides oxidation inhibition, other parameters such as rust and wear control are also important.

A major challenge in engine oil formulation is simultaneously achieving improved fuel economy while also achieving appropriate solubility and dispersibility for polar additives or sludge generated during service of lubricating oils and oxidative stability.

Therefore, there is need for better additive and base stock technology for lubricant compositions that will meet ever more stringent requirements of lubricant users. In particular, there is a need for advanced additive technology and synthetic base stocks with improved fuel economy, low temperature properties, solubility and dispersibility for polar additives or sludge generated during service of lubricating oils, and oxidative stability.

The present disclosure also provides many additional advantages, which shall become apparent as described below.

## SUMMARY

This disclosure provides compositions that include one or more monoester base stocks of monomethyl branched alcohols and linear aliphatic acids that have desirable low viscosity/low volatility properties and high viscosity index. Viscosity Index (VI) indicates the ability of the lubricant to maintain a film between moving parts at high temperatures. VI is the measure of the rate of change of a lubricant's viscosity as temperature of the lubricant changes. The lower the rate viscosity change, the higher the VI. Thus fluids with higher viscosity index have substantially higher benefits than lower viscosity index basestocks. Thus, the lubricating oil base stocks of this disclosure provide a solution to achieve enhanced fuel economy and energy efficiency. In addition, good solvency for commonly used polar additives and potentially good hydrolytic, thermal and oxidative stability, deposit control and traction control are other advantages of these compositions.

This disclosure relates in part to a monomethyl ester composition comprising one or more compounds represented by the formula



wherein R<sub>1</sub> is a monomethyl branched C<sub>15</sub> to C<sub>19</sub> alkyl group and R<sub>2</sub> is an unsubstituted C<sub>2</sub> to C<sub>30</sub> linear alkyl group. The composition has a viscosity (K<sub>v100</sub>) from about 1 cSt to about 10 cSt at 100° C. as determined by ASTM D445, a viscosity index (VI) from about -100 to about 300 as determined by ASTM D2270, and a Noack volatility of no greater than 50 percent as determined by ASTM D5800.

This disclosure also relates in part to a monomethyl ester composition comprising one or more compounds represented by the formula



wherein R<sub>1</sub> is a monomethyl branched C<sub>15</sub> to C<sub>19</sub> alkyl group and R<sub>2</sub> is an unsubstituted C<sub>2</sub> to C<sub>30</sub> linear alkyl group. The composition has a viscosity (K<sub>v100</sub>) from about 1 cSt to about 10 cSt at 100° C. as determined by ASTM D445, a viscosity index (VI) from about -100 to about 300 as determined by ASTM D2270, a pour points from about 0° C. to about -50° C. as determined by ASTM D97, and a Noack volatility of no greater than 50 percent as determined by ASTM D5800. The one or more compounds are produced by a process comprising reacting a monomethyl substituted C<sub>15</sub> to C<sub>19</sub> linear alcohol with an unsubstituted C<sub>2</sub> to C<sub>30</sub> linear aliphatic acid, optionally in the presence of a catalyst and a solvent, under reaction conditions sufficient to produce said one or more compounds.

This disclosure further relates in part to a lubricating oil base stock comprising one or more compounds represented by the formula



5

wherein R<sub>1</sub> is a monomethyl branched C<sub>15</sub> to C<sub>19</sub> alkyl group and R<sub>2</sub> is an unsubstituted C<sub>2</sub> to C<sub>30</sub> linear alkyl group. The base stock has a viscosity (K<sub>v100</sub>) from about 1 cSt to about 10 cSt at 100° C. as determined by ASTM D445, a viscosity index (VI) from about -100 to about 300 as determined by ASTM D2270, a pour points from about 0° C. to about -50° C. as determined by ASTM D97, and a Noack volatility of no greater than 50 percent as determined by ASTM D5800.

This disclosure yet further relates in part to a lubricating oil comprising a lubricating oil base stock component, and a monoester cobase stock component; wherein said monoester cobase stock comprises one or more compounds represented by the formula



wherein R<sub>1</sub> is a monomethyl branched C<sub>15</sub> to C<sub>19</sub> alkyl group and R<sub>2</sub> is an unsubstituted C<sub>2</sub> to C<sub>30</sub> linear alkyl group. The composition has a viscosity (K<sub>v100</sub>) from about 1 cSt to about 10 cSt at 100° C. as determined by ASTM D445, a viscosity index (VI) from about -100 to about 300 as determined by ASTM D2270, and a Noack volatility of no greater than 50 percent as determined by ASTM D5800.

This disclosure also relates in part to a method for improving one or more of cold flow properties, thermal and oxidative stability, solubility and dispersancy of polar additives, deposit control and traction control in a lubricating oil by using as the lubricating oil a formulated oil comprising a lubricating oil base stock as a major component, and a monoester cobase stock as a minor component; wherein said monoester cobase stock comprises one or more compounds represented by the formula



40

wherein R<sub>1</sub> is a monomethyl branched C<sub>15</sub> to C<sub>19</sub> alkyl group and R<sub>2</sub> is an unsubstituted C<sub>2</sub> to C<sub>30</sub> linear alkyl group, and wherein said lubricating oil has a viscosity (K<sub>v100</sub>) from about 1 cSt to about 10 cSt at 100° C. as determined by ASTM D445, a viscosity index (VI) from about -100 to about 300 as determined by ASTM D2270, a pour points from about 0° C. to about -50° C. as determined by ASTM D97, and a Noack volatility of no greater than 50 percent as determined by ASTM D5800. The lubricating oil is used in a formulated oil to improve one or more of cold flow properties, thermal and oxidative stability, solubility and dispersancy of polar additives, deposit control and traction control.

This disclosure also relates to a lubricating oil base stock comprising one or more compounds represented by the formula



65

wherein R<sub>1</sub> is a monomethyl branched C<sub>15</sub> to C<sub>19</sub> alkyl group and R<sub>2</sub> is selected from the group consisting of a substituted or unsubstituted aryl group (C<sub>4</sub>-C<sub>30</sub>), heteroaryl group (C<sub>4</sub>-C<sub>30</sub>), arylalkyl group (C<sub>5</sub>-C<sub>30</sub>) and alkoxy group (C<sub>1</sub>-C<sub>30</sub>), and wherein said base stock has a viscosity (K<sub>V100</sub>) from about 1 cSt to about 10 cSt at 100° C. as determined by ASTM D445, a viscosity index (VI) from about -100 to about 300 as determined by ASTM D2270, a pour points from about 0° C. to about -50° C. as determined by ASTM D97, and a Noack volatility of no greater than 50 percent as determined by ASTM D5800, wherein said one or more compounds are produced by a process comprising reacting a monomethyl substituted C<sub>15</sub> to C<sub>19</sub> linear alcohol with a carboxylic acid, an aromatic alkanoic acid, or a glycol ether acid, optionally in the presence of a catalyst and a solvent, under reaction conditions sufficient to produce said one or more compounds.

It has been surprisingly found that outstanding viscosity index and pour point properties, low viscosity low volatility properties, good high-temperature thermal and oxidative stability, good solvency for polar additives, deposit control, and traction benefits, can be attained in an engine lubricated with a lubricating oil by using as the lubricating oil a formulated oil in accordance with this disclosure. In particular, a lubricating oil base stock comprising one or more monomethyl esters exhibits low viscosity, low volatility, good cold flow properties, desired solvency for polar additives, superior oxidative stability, desired deposit control and traction benefits, which helps to prolong the useful life of lubricants and significantly improve the durability and resistance of lubricants when exposed to high temperatures. The lubricating oils of this disclosure are particularly advantageous as passenger vehicle engine oil (PVEO) products.

Further objects, features and advantages of the present disclosure will be understood by reference to the following drawings and detailed description.

#### DETAILED DESCRIPTION

All numerical values within the detailed description and the claims herein are modified by "about" or "approximately" the indicated value, and take into account experimental error and variations that would be expected by a person having ordinary skill in the art.

The compositions of this disclosure are near linear, low viscosity, low volatility monomethyl esters of monomethyl branched alcohols and linear aliphatic acids. These compositions exhibit (1) outstanding low viscosity low volatility properties, (2) good high-temperature thermal and oxidative stability, (3) good solvency for polar additives, (4) good deposit control, (4) good low temperature properties, and (5) traction benefits, which make them attractive as Group V synthetic base stocks in high performance, fuel economy lubricant applications.

Low viscosity base stocks (e.g., kinematic viscosity at 100° C., 2-3 cSt) currently available in the marketplace are too volatile (Noack>15-20%) to be used for formulating next-generation ultra-low viscosity engine oils (i.e., xxW-4->xxW-16). These base stocks (e.g., SpectraSyn™ 2, QHVTM 3, bis-(2-ethylhexyl) adipate, di-2-ethylhexyl azelate, Esterex™ A32) are unable to provide formulated engine oils that also meet current volatility API specification. In addition, current Group V ester base stocks generally have poor high temperature oxidation stability which can cause operational problems in engine, potentially causing high deposit formation. The present disclosure identifies near linear monoesters that have desirable low viscosity and

low volatility properties while exhibiting traction benefits, good low temperature properties, good deposit control behavior and good high-temperature thermal-oxidative stability, hence provides a solution to achieve enhanced fuel economy and energy efficiency. In addition, good solvency for commonly used polar additives and potentially good hydrolytic stability are other advantages of these compounds in base stock applications.

As indicated above, the compositions of this disclosure include, for example, one or more monomethyl ester compounds represented by the formula



wherein R<sub>1</sub> is a monomethyl branched C<sub>15</sub> to C<sub>19</sub> alkyl

group and R<sub>2</sub> is an unsubstituted C<sub>2</sub> to C<sub>30</sub> linear alkyl group. The composition has a viscosity (K<sub>V100</sub>) from about 1 cSt to about 10 cSt at 100° C. as determined by ASTM D445, a viscosity index (VI) from about -100 to about 300 as determined by ASTM D2270, a pour points from about 0° C. to about -50° C. as determined by ASTM D97, and a Noack volatility of no greater than 50 percent as determined by ASTM D5800.

Preferred compositions of this disclosure include, for example, those wherein R<sub>2</sub> is an unsubstituted C<sub>2</sub> to C<sub>10</sub> linear alkyl group, or an unsubstituted C<sub>5</sub> to C<sub>9</sub> linear alkyl group. In addition, R<sub>1</sub> may be a monomethyl branched C<sub>15</sub> alkyl, a monomethyl branched C<sub>16</sub> alkyl, a monomethyl branched C<sub>17</sub> alkyl, monomethyl branched C<sub>15</sub> alkyl, monomethyl branched C<sub>19</sub> alkyl, or a combination thereof.

Alternative composition of this disclosure include, for example, those wherein R<sub>2</sub> is a substituted or unsubstituted aryl group (C<sub>4</sub>-C<sub>30</sub>), a substituted or unsubstituted heteroaryl group (C<sub>4</sub>-C<sub>30</sub>), a substituted or unsubstituted arylalkyl group (C<sub>5</sub>-C<sub>30</sub>) and a substituted or unsubstituted alkoxy group (C<sub>1</sub>-C<sub>30</sub>).

Particularly preferred monomethyl ester compounds of the instant disclosure include 8-methylpentadecyl hexanoate, 8-methylpentadecyl octanoate, 8-methylpentadecyl decanoate, and combinations thereof.

Illustrative monomethyl ester compositions of this disclosure have a viscosity (K<sub>V100</sub>) from about 1 cSt to about 8 cSt, more preferably from about 2 cSt to about 6 cSt, at 100° C. as determined by ASTM D445 or ASTM D7042, a viscosity index (VI) from about -100 to about 300, more preferably from about 0 to about 200, even more preferably from about 25 to about 150, as determined by ASTM D2270, a pour point of from about 0° C. to about -50° C., more preferably from about -20° C. to about -50° C. even more preferably from about -30° C. to about -50° C. as determined by ASTM D97, a Noack volatility of no greater than 90 percent, more preferably no greater than 50 percent, even more preferably no greater than 30 percent, still even more preferably no greater than 15 percent, as determined by ASTM D5800.

The monomethyl ester compositions of this disclosure can be prepared by a process that involves reacting a monomethyl substituted C<sub>15</sub> to C<sub>19</sub> linear alcohol, or more preferably a C<sub>16</sub> to C<sub>17</sub> linear alcohol with an acid, optionally in the presence of a catalyst and a solvent, under reaction conditions sufficient to produce said compositions.

The monomethyl substituted C<sub>15</sub> to C<sub>19</sub> linear alcohol useful in the process of the present disclosure for making the near-linear hexanoate, near-linear octanoate and near-linear

decanoate esters are sold under the trade name Neodol 67 by Shell Chemical Co. (Houston, Tex.) and may be represented by the following formula:

Branched Monomethyl C<sub>16</sub> Alcohol with Branching at Eighth Carbon



Branched Monomethyl C<sub>17</sub> Alcohol with Branching at Ninth Carbon



In the above formula, branching in the monomethyl branched C<sub>16</sub> and C<sub>17</sub> alcohol may vary from the second carbon to the fourteenth or fifteenth carbon in the linear chain. More particularly, the methyl branch may occur at the second, or third, or fourth, or fifth, or sixth, or seventh, or eighth, or ninth, or tenth, or eleventh, or twelfth, or thirteenth, or fourteenth, or fifteenth carbon of the linear chain.

The preferred chain distribution of the Neodol 67 alcohol is shown in Table 1 below.

TABLE 1

|     | Preferred Range | Narrow Preferred Range | Typical Preferred Range |
|-----|-----------------|------------------------|-------------------------|
| C15 | 2%-5%           | 2%                     | 2%                      |
| C16 | 28%-48%         | 33%-43%                | 38%                     |
| C17 | 33%-73%         | 43%-63%                | 53%                     |
| C18 | 4%-12%          | 6%-10%                 | 6%                      |
| C19 | 1%-5%           | 0%-4%                  | 1%                      |

The acids of the present disclosure may be an aliphatic acid, or a carboxylic acid, or an aromatic alkanoic acid, or a glycol ether acid, or a combination thereof.

Illustrative aliphatic acids useful in the process of this disclosure include, for example, valeric acid, isovaleric acid, hexanoic acid, heptanoic acid, 2-ethylhexanoic acid, octanoic acid, isoctanoic acid, nonanoic acid, isononanoic acid, decanoic acid, isodecanoic acid, undecanoic acid, dodecanoic acid, tridecanoic acid, isotridecanoic acid, tetradecanoic acid, hexadecanoic acid, stearic acid, isostearic acid, and the like.

Illustrative carboxylic acids useful in the process of this disclosure include, for example, isobutyric acid, 2-ethylhexanoic acid, 2-butylhexanoic acid, 2-butyloctanoic acid, 2-hexyldecanoic acid, 2-heptylundecanoic acid, 2-octyldecanoic acid, 2-decyldodecanoic acid, isotridecanoic acid, and the like.

Illustrative aromatic alkanoic acids useful in the process of this disclosure include, for example, benzoic acid, phenylacetic acid, phenylpropionic acid, phenylbutyric acid, methoxyphenylacetic acid, tolylacetic acid, nitrophenylacetic acid, xylylacetic acid, tolylpropionic acid, xylylpropionic acid, methoxyphenylpropionic acid, methoxyphenyl-

butyric acid, nitrophenylpropionic acid, nitrophenylbutyric acid, xylylbutyric acid, tolylbutyric acid, and the like.

Illustrative glycol ether acids useful in the process of this disclosure include, for example, methoxyacetic acid, methoxypropionic acid, methoxyethoxyacetic acid, methoxyethoxyethoxyacetic acid, ethoxyacetic acid, ethoxyethoxyacetic acid, ethoxyethoxyethoxyacetic acid, propoxyacetic acid, propoxyethoxyacetic acid, propoxyethoxyethoxyacetic acid, butoxyacetic acid, butoxyethoxyacetic acid, butoxyethoxyethoxyacetic acid, propoxybenzoic acid, and the like.

Reaction conditions for the reaction of the alcohol with the acid, such as temperature, pressure and contact time, may also vary greatly and any suitable combination of such conditions may be employed herein. The reaction temperature may range between about 25° C. to about 300° C., and preferably between about 50° C. to about 250° C., and more preferably between about 100° C. to about 200° C. Normally the reaction is carried out under ambient pressure and the contact time may vary from a matter of seconds or minutes to a few hours or greater. The reactants can be added to the reaction mixture or combined in any order. The reaction residence time employed can range from about 30 seconds to about 48 hours, preferably from about 5 minutes to 36 hours, and more preferably from about 1 hour to 24 hours.

As shown in the Examples herein, the monomethyl ester compositions have more desirable viscosity-volatility characteristics when compared to commercially available low viscosity Group IV PAO synthetic base stocks (e.g., SpectraSn™ 2, SpectraSyn™ 4) or Group V ester base stocks (e.g., 2-ethylhexyl oleate, 2-ethylhexyl adipate, isodecyl adipate, 2-ethylhexyl phthalate, nC8/nC10 neopentyl glycol esters, nC7 trimethylolpropane ester, and the like). As shown in the Examples herein, the monomethyl ester compositions of the present disclosure have lower viscosities than commercially available esters at similar volatility. Additionally, the monomethyl ester compositions of the present disclosure have lower volatility than commercially available esters at comparable viscosities and good low temperature properties as measured by pour point and Viscosity Index.

Furthermore, it has been found that these monomethyl ester compositions also show high solvency for the typical additive components (e.g., antiwear additives, friction modifiers, dispersants, detergents, antioxidants, viscosity modifiers, pour point depressants, antifoaming agent, etc.) employed in the formulation of PVL (Passenger Vehicles Lubricants), CVL (Commercial Vehicles Lubricants), as well as industrial applications.

Examples of techniques that can be employed to characterize the compositions formed by the process described above include, but are not limited to, analytical gas chromatography, nuclear magnetic resonance, thermogravimetric analysis (TGA), inductively coupled plasma mass spectrometry, differential scanning calorimetry (DSC), volatility and viscosity measurements.

This disclosure provides lubricating oils useful as engine oils and in other applications characterized by excellent oxidative stability. The lubricating oils are based on high quality base stocks including a major portion of a hydrocarbon base fluid such as a PAO or GTL with a secondary cobase stock component which is a monoester as described herein. The lubricating oil base stock can be any oil boiling in the lube oil boiling range, typically between about 100 to 450° C. In the present specification and claims, the terms base oil(s) and base stock(s) are used interchangeably.

The viscosity-temperature relationship of a lubricating oil is one of the critical criteria which must be considered when

selecting a lubricant for a particular application. Viscosity Index (VI) is an empirical, unitless number which indicates the rate of change in the viscosity of an oil within a given temperature range. Fluids exhibiting a relatively large change in viscosity with temperature are said to have a low viscosity index. A low VI oil, for example, will thin out at elevated temperatures faster than a high VI oil. Usually, the high VI oil is more desirable because it has higher viscosity at higher temperature, which translates into better or thicker lubrication film and better protection of the contacting machine elements.

In another aspect, as the oil operating temperature decreases, the viscosity of a high VI oil will not increase as much as the viscosity of a low VI oil. This is advantageous because the excessive high viscosity of the low VI oil will decrease the efficiency of the operating machine. Thus high VI (HVI) oil has performance advantages in both high and low temperature operation. VI is determined according to ASTM D2270. VI is related to kinematic viscosities measured at 40° C. and 100° C. using ASTM D445.

#### Lubricating Oil Base Stocks

A wide range of lubricating oils is known in the art. Lubricating oils that are useful in the present disclosure are both natural oils and synthetic oils. Natural and synthetic oils (or mixtures thereof) can be used unrefined, refined, or rerefined (the latter is also known as reclaimed or reprocessed oil). Unrefined oils are those obtained directly from a natural or synthetic source and used without added purification. These include shale oil obtained directly from retorting operations, petroleum oil obtained directly from primary distillation, and ester oil obtained directly from an esterification process. Refined oils are similar to the oils discussed for unrefined oils except refined oils are subjected to one or more purification steps to improve the at least one lubricating oil property. One skilled in the art is familiar with many purification processes. These processes include solvent extraction, secondary distillation, acid extraction, base extraction, filtration, and percolation. Rerefined oils are obtained by processes analogous to refined oils but using an oil that has been previously used as a feed stock.

Groups I, II, III, IV and V are broad categories of base oil stocks developed and defined by the American Petroleum Institute (API Publication 1509; [www.API.org](http://www.API.org)) to create guidelines for lubricant base oils. Group I base stocks generally have a viscosity index of between about 80 to 120 and contain greater than about 0.03% sulfur and less than about 90% saturates. Group II base stocks generally have a viscosity index of between about 80 to 120, and contain less than or equal to about 0.03% sulfur and greater than or equal to about 90% saturates. Group III stock generally has a viscosity index greater than about 120 and contains less than or equal to about 0.03% sulfur and greater than about 90% saturates. Group IV includes polyalphaolefins (PAO). Group V base stocks include base stocks not included in Groups I-IV. Table 2 below summarizes properties of each of these five groups.

TABLE 2

| Base Oil Properties |            |                 |
|---------------------|------------|-----------------|
| Saturates           | Sulfur     | Viscosity Index |
| Group I <90 and/or  | >0.03% and | ≥80 and <120    |
| Group II ≥90 and    | ≤0.03% and | ≥80 and <120    |
| Group III ≥90 and   | ≤0.03% and | ≥120            |

TABLE 2-continued

| Base Oil Properties |                                                                   |                                          |                 |
|---------------------|-------------------------------------------------------------------|------------------------------------------|-----------------|
|                     | Saturates                                                         | Sulfur                                   | Viscosity Index |
| 5 Group IV          |                                                                   | Includes polyalphaolefins (PAO) products |                 |
| Group V             | All other base oil stocks not included in Groups I, II, III or IV |                                          |                 |

10 Natural oils include animal oils, vegetable oils (castor oil and lard oil, for example), and mineral oils. Animal and vegetable oils possessing favorable thermal oxidative stability can be used. Of the natural oils, mineral oils are preferred. Mineral oils vary widely as to their crude source, for example, as to whether they are paraffinic, naphthenic, or mixed paraffinic-naphthenic. Oils derived from coal or shale are also useful in the present disclosure. Natural oils vary also as to the method used for their production and purification, for example, their distillation range and whether they are straight run or cracked, hydrorefined, or solvent extracted.

15 Group II and/or Group III hydroprocessed or hydrocracked base stocks, as well as synthetic oils such as polyalphaolefins, alkyl aromatics and synthetic esters, i.e. Group IV and to Group V oils are also well known base stock oils.

20 Synthetic oils include hydrocarbon oil such as polymerized and interpolymerized olefins (polybutylenes, polypropylenes, propylene isobutylene copolymers, ethylene-olefin copolymers, and ethylene-alphaolefin copolymers, for example). Polyalphaolefin (PAO) oil base stocks, the Group 25 IV API base stocks, are a commonly used synthetic hydrocarbon oil. By way of example, PAOs derived from C<sub>8</sub>, C<sub>10</sub>, C<sub>12</sub>, C<sub>14</sub> olefins or mixtures thereof may be utilized. See U.S. Pat. Nos. 4,956,122; 4,827,064; and 4,827,073, which are incorporated herein by reference in their entirety. Group 30 IV oils, that is, the PAO base stocks have viscosity indices preferably greater than 130, more preferably greater than 135, still more preferably greater than 140.

25 Esters may be useful in the lubricating oils of this disclosure. Additive solvency and seal compatibility characteristics may be secured by the use of esters such as the esters of dibasic acids with monoalkanols and the polyol esters of monocarboxylic acids. Esters of the former type include, for example, the esters of dicarboxylic acids such as phthalic acid, succinic acid, sebacic acid, fumaric acid, adipic acid, linoleic acid dimer, malonic acid, alkyl malonic acid, alk-40 enyl malonic acid, etc., with a variety of alcohols such as butyl alcohol, hexyl alcohol, dodecyl alcohol, 2-ethylhexyl alcohol, etc. Specific examples of these types of esters include dibutyl adipate, di(2-ethylhexyl) sebacate, di-n-50 hexyl fumarate, dioctyl sebacate, diisooctyl azelate, diisooctyl azelate, dioctyl phthalate, didecyl phthalate, dieicosyl sebacate, etc.

35 Particularly useful synthetic esters are those which are obtained by reacting one or more polyhydric alcohols, 55 preferably the hindered polyols such as the neopentyl polyols: e.g., neopentyl glycol, trimethylol ethane, 2-methyl-2-propyl-1,3-propanediol, trimethylol propane, pentaerythritol and dipentaerythritol with alkanoic acids containing at least about 4 carbon atoms, preferably C<sub>5</sub> to C<sub>30</sub> acids such as 60 saturated straight chain fatty acids including caprylic acid, capric acids, lauric acid, myristic acid, palmitic acid, stearic acid, arachic acid, and behenic acid, or the corresponding branched chain fatty acids or unsaturated fatty acids such as oleic acid, or mixtures of any of these materials.

65 Esters should be used in an amount such that the improved wear and corrosion resistance provided by the lubricating oils of this disclosure are not adversely affected.

## 11

Non-conventional or unconventional base stocks and/or base oils include one or a mixture of base stock(s) and/or base oil(s) derived from: (1) one or more Gas-to-Liquids (GTL) materials, as well as (2) hydrodewaxed, or hydroisomerized/cat (and/or solvent) dewaxed base stock(s) and/or base oils derived from synthetic wax, natural wax or waxy feeds, mineral and/or non-mineral oil waxy feed stocks such as gas oils, slack waxes (derived from the solvent dewaxing to of natural oils, mineral oils or synthetic oils, e.g., Fischer-Tropsch feed stocks), natural waxes, and waxy stocks such as gas oils, waxy fuels hydrocracker bottoms, waxy raffinate, hydrocrackate, thermal crackates, foot oil or other mineral, mineral oil, or even non-petroleum oil derived waxy materials such as waxy materials recovered from coal liquefaction or shale oil, linear or branched hydrocarbyl compounds with carbon number of about 20 or greater, preferably about 30 or greater and mixtures of such base stocks and/or base oils.

GTL materials are materials that are derived via one or more synthesis, combination, transformation, rearrangement, and/or degradation/deconstructive processes from gaseous carbon-containing compounds, hydrogen-containing compounds and/or elements as feed stocks such as hydrogen, carbon dioxide, carbon monoxide, water, methane, ethane, ethylene, acetylene, propane, propylene, propyne, butane, butylenes, and butynes. GTL base stocks and/or base oils are GTL materials of lubricating viscosity that are generally derived from hydrocarbons; for example, waxy synthesized hydrocarbons, that are themselves derived from simpler gaseous carbon-containing compounds, hydrogen-containing compounds and/or elements as feed stocks. GTL base stock(s) and/or base oil(s) include oils boiling in the lube oil boiling range (1) separated/fractionated from synthesized GTL materials such as, for example, by distillation and subsequently subjected to a final wax processing step which involves either or both of a catalytic dewaxing process, or a solvent dewaxing process, to produce lube oils of reduced/low pour point; (2) synthesized wax isomers, comprising, for example, hydrodewaxed or hydroisomerized cat and/or solvent dewaxed synthesized wax or waxy hydrocarbons; (3) hydrodewaxed or hydroisomerized cat and/or solvent dewaxed Fischer-Tropsch (F-T) material (i.e., hydrocarbons, waxy hydrocarbons, waxes and possible analogous oxygenates); preferably hydrodewaxed or hydroisomerized/followed by cat and/or solvent dewaxing dewaxed F-T waxy hydrocarbons, or hydrodewaxed or hydroisomerized/followed by cat (or solvent) dewaxing dewaxed, F-T waxes, or mixtures thereof.

GTL base stock(s) and/or base oil(s) derived from GTL materials, especially, hydrodewaxed or hydroisomerized/ followed by cat and/or solvent dewaxed wax or waxy feed, preferably F-T material derived base stock(s) and/or base oil(s), are characterized typically as having kinematic viscosities at 100° C. of from about 2 mm<sup>2</sup>/s to about 50 mm<sup>2</sup>/s (ASTM D445). They are further characterized typically as having pour points of -5° C. to about -40° C. or lower (ASTM D97). They are also characterized typically as having viscosity indices of about 80 to about 140 or greater (ASTM D2270).

In addition, the GTL base stock(s) and/or base oil(s) are typically highly paraffinic (>90% saturates), and may contain mixtures of monocycloparaffins and multicycloparaffins in combination with non-cyclic isoparaffins. The ratio of the naphthenic (i.e., cycloparaffin) content in such combinations varies with the catalyst and temperature used. Further, GTL base stock(s) and/or base oil(s) typically have very low sulfur and nitrogen content, generally containing less than

## 12

about 10 ppm, and more typically less than about 5 ppm of each of these elements. The sulfur and nitrogen content of GTL base stock(s) and/or base oil(s) obtained from F-T material, especially F-T wax, is essentially nil. In addition, the absence of phosphorous and aromatics make this material especially suitable for the formulation of low SAP products.

The term GTL base stock and/or base oil and/or wax isomerate base stock and/or base oil is to be understood as embracing individual fractions of such materials of wide viscosity range as recovered in the production process, mixtures of two or more of such fractions, as well as mixtures of one or two or more low viscosity fractions with one, two or more higher viscosity fractions to produce a blend wherein the blend exhibits a target kinematic viscosity.

The GTL material, from which the GTL base stock(s) and/or base oil(s) is/are derived is preferably an F-T material (i.e., hydrocarbons, waxy hydrocarbons, wax).

Base oils for use in the formulated lubricating oils useful in the present disclosure are any of the variety of oils corresponding to API Group I, Group II, Group III, Group IV, Group V and Group VI oils and mixtures thereof, preferably API Group II, Group III, Group IV, Group V and Group VI oils and mixtures thereof, more preferably the Group III to Group VI base oils due to their exceptional volatility, stability, viscometric and cleanliness features. Minor quantities of Group I stock, such as the amount used to dilute additives for blending into formulated lube oil products, can be tolerated but should be kept to a minimum, i.e. amounts only associated with their use as diluent/carrier oil for additives used on an "as received" basis. Even in regard to the Group II stocks, it is preferred that the Group II stock be in the higher quality range associated with that stock, i.e. a Group II stock having a viscosity index in the range 100<VI<120.

In addition, the GTL base stock(s) and/or base oil(s) are typically highly paraffinic (>90% saturates), and may contain mixtures of monocycloparaffins and multicycloparaffins in combination with non-cyclic isoparaffins. The ratio of the naphthenic (i.e., cycloparaffin) content in such combinations varies with the catalyst and temperature used. Further, GTL base stock(s) and/or base oil(s) and hydrodewaxed, or hydroisomerized/cat (and/or solvent) dewaxed base stock(s) and/or base oil(s) typically have very low sulfur and nitrogen content, generally containing less than about 10 ppm, and more typically less than about 5 ppm of each of these elements. The sulfur and nitrogen content of GTL base stock(s) and/or base oil(s) obtained from F-T material, especially F-T wax, is essentially nil. In addition, the absence of phosphorous and aromatics make this material especially suitable for the formulation of low sulfur, sulfated ash, and phosphorus (low SAP) products.

The base stock component of the present lubricating oils will typically be from 1 to 99 weight percent of the total composition (all proportions and percentages set out in this specification are by weight unless the contrary is stated) and more preferably in the range of 10 to 99 weight percent, or more preferably from 15 to 80 percent, or more preferably from 20 to 70 percent, or more preferably from 25 to 60 percent, or more preferably from 30 to 50 percent. Monomethyl Ester Base Stock and Cobase Stock Components

The monomethyl ester base stock and cobase stock components useful in this disclosure include, for example, compositions containing one or more compounds represented by the formula



wherein  $\text{R}_1$  is a monomethyl branched  $\text{C}_{15}$  to  $\text{C}_{11}$  alkyl group and  $\text{R}_2$  is an unsubstituted  $\text{C}_2$  to  $\text{C}_{30}$  linear alkyl group. The composition has a viscosity ( $\text{Kv}_{100}$ ) from about 1 cSt to about 10 cSt at 100° C. as determined by ASTM D445, a viscosity index (VI) from about -100 to about 300 as determined by ASTM D2270, a pour points from about 0° C. to about -50° C. as determined by ASTM D97, and a Noack volatility of no greater than 50 percent as determined by ASTM D5800.

Preferred monomethyl ester base stock and cobase stock components of this disclosure include, for example, those wherein  $\text{R}_2$  is an unsubstituted  $\text{C}_2$  to  $\text{C}_{10}$  linear alkyl group, or an unsubstituted  $\text{C}_5$  to  $\text{C}_9$  linear alkyl group. In addition,  $\text{R}_1$  may be a monomethyl branched  $\text{C}_{15}$  alkyl, a monomethyl branched  $\text{C}_{16}$  alkyl, a monomethyl branched  $\text{C}_{17}$  alkyl, a monomethyl branched  $\text{C}_{15}$  alkyl, monomethyl branched  $\text{C}_{19}$  alkyl, or a combination thereof.

Alternative monomethyl ester base stock and cobase stock components of this disclosure include, for example, those wherein  $\text{R}_2$  is a substituted or unsubstituted aryl group ( $\text{C}_4\text{-C}_{30}$ ), a substituted or unsubstituted heteroaryl group ( $\text{C}_4\text{-C}_{30}$ ), a substituted or unsubstituted arylalkyl group ( $\text{C}_5\text{-C}_{30}$ ) and a substituted or unsubstituted alkoxy group ( $\text{C}_1\text{-C}_{30}$ ).

Particularly preferred monomethyl ester base stock and cobase stock components of the instant disclosure include 8-methylpentadecyl hexanoate, 8-methylpentadecyl octanoate, 8-methylpentadecyl decanoate, and combinations thereof.

Illustrative monomethyl ester base stock and cobase stock components of this disclosure have a viscosity ( $\text{Kv}_{100}$ ) from about 1 cSt to about 8 cSt, more preferably from about 2 cSt to about 6 cSt, at 100° C. as determined by ASTM D445 or ASTM D7042, a viscosity index (VI) from about -100 to about 300, more preferably from about 0 to about 200, even more preferably from about 25 to about 150, as determined by ASTM D2270, a pour point of from about 0° C. to about -50° C., more preferably from about -20° C. to about -50° C., even more preferably from about -30° C. to about -50° C. as determined by ASTM D97, a Noack volatility of no greater than 90 percent, more preferably no greater than 50 percent, even more preferably no greater than 30 percent, still even more preferably no greater than 15 percent, as determined by ASTM D5800, and a high temperature high shear (HTHS) viscosity of less than about 2.5 cP, more preferably less than about 2.25 cP, even more preferably less than about 2.0 cP, as determined by ASTM D4683.

The monomethyl ester base stock and cobase stock components of this disclosure can be prepared by a process that involves reacting a monomethyl substituted  $\text{C}_{15}$  to  $\text{C}_{19}$  linear alcohol, or more preferably a  $\text{C}_{16}$  to  $\text{C}_{17}$  linear alcohol with an acid, optionally in the presence of a catalyst and a solvent, under reaction conditions sufficient to produce said compositions.

The monomethyl substituted  $\text{C}_{15}$  to  $\text{C}_{19}$  linear alcohol useful in the process of the present disclosure for making the near-linear hexanoate, near-linear octanoate and near-linear decanoate esters are sold under the trade name Neodol 67 by Shell Chemical Co. (Houston, Tex.).

The monomethyl substituted  $\text{C}_1$  to  $\text{C}_{19}$  linear alcohol useful in the process of the present disclosure for making the

near-linear hexanoate, near-linear octanoate and near-linear decanoate esters are sold under the trade name Neodol 67 by Shell Chemical Co. (Houston, Tex.) and may be represented by the following formula:

Branched Monomethyl  $\text{C}_{16}$  Alcohol with Branching at Eighth Carbon



Branched Monomethyl  $\text{C}_{17}$  Alcohol with Branching at Ninth Carbon



In the above formula, branching in the monomethyl branched  $\text{C}_{16}$  and  $\text{C}_{17}$  alcohol may vary from the second carbon to the fourteenth or fifteenth carbon in the linear chain. More particularly, the methyl branch may occur at the second, or third, or fourth, or fifth, or sixth, or seventh, or eighth, or ninth, or tenth, or eleventh, or twelfth, or thirteenth, or fourteenth, or fifteenth carbon of the linear chain.

The preferred chain distribution of the Neodol 67 alcohol is shown in Table 3 below.

TABLE 3

|     | Preferred Range | Narrow Preferred Range | Typical Preferred Range |
|-----|-----------------|------------------------|-------------------------|
| C15 | 2%-5%           | 2%                     | 2%                      |
| C16 | 28%-48%         | 33%-43%                | 38%                     |
| C17 | 33%-73%         | 43%-63%                | 53%                     |
| C18 | 4%-12%          | 6%-10%                 | 6%                      |
| C19 | 1%-5%           | 0%-4%                  | 1%                      |

The acids of the present disclosure may be an aliphatic acid, or a carboxylic acid, or an aromatic alkanoic acid, or a glycol ether acid, or a combination thereof.

Illustrative aliphatic acids useful in the process of this disclosure include, for example, valeric acid, isovaleric acid, hexanoic acid, heptanoic acid, 2-ethylhexanoic acid, octanoic acid, isoctanoic acid, nonanoic acid, isononanoic acid, decanoic acid, isodecanoic acid, undecanoic acid, dodecanoic acid, tridecanoic acid, isotridecanoic acid, tetradecanoic acid, hexadecanoic acid, stearic acid, isostearic acid, and the like.

Illustrative carboxylic acids useful in the process of this disclosure include, for example, isobutyric acid, 2-ethylhexanoic acid, 2-butylhexanoic acid, 2-butyloctanoic acid, 2-hexyldecanoic acid, 2-heptylundecanoic acid, 2-octyldecanoic acid, 2-decyldodecanoic acid, isotridecanoic acid, and the like.

Illustrative aromatic alkanoic acids useful in the process of this disclosure include, for example, benzoic acid, phenylacetic acid, phenylpropionic acid, phenylbutyric acid, methoxyphenylacetic acid, tolylacetica acid, nitrophenylacetic acid, xylylacetica acid, tolylpropionic acid, xylylpropionic acid, methoxyphenylpropionic acid, methoxyphenyl-

## 15

butyric acid, nitrophenylpropionic acid, nitrophenylbutyric acid, xylolbutyric acid, tolylbutyric acid, and the like.

Illustrative glycol ether acids useful in the process of this disclosure include, for example, methoxyacetic acid, methoxypropionic acid, methoxyethoxyacetic acid, methoxyethoxyethoxyacetic acid, ethoxyacetic acid, ethoxyethoxyacetic acid, ethoxethoxyethoxyacetic acid, propoxyacetic acid, propoxyethoxyacetic acid, propoxyethoxyethoxyacetic acid, butoxyacetic acid, butoxyethoxyacetic acid, butoxyethoxyethoxyacetic acid, propoxyethoxyethoxyacetic acid, and the like.

Reaction conditions for the reaction of the alcohol with the acid, such as temperature, pressure and contact time, may also vary greatly and any suitable combination of such conditions may be employed herein. The reaction temperature may range between about 25° C. to about 300° C., and preferably between about 50° C. to about 250° C., and more preferably between about 100° C. to about 200° C. Normally the reaction is carried out under ambient pressure and the contact time may vary from a matter of seconds or minutes to a few hours or greater. The reactants can be added to the reaction mixture or combined in any order. The reaction residence time employed can range from about 30 seconds to about 48 hours, preferably from about 5 minutes to 36 hours, and more preferably from about 1 hour to 24 hours.

The monomethyl ester base stock component is preferably present in an amount sufficient for providing oxidative stability in the lubricating oil. The monoester base stock component can be present as the major base stock in the lubricating oils of this disclosure. Accordingly, the monoester can be present in an amount from about 1 to about 99 weight percent, preferably from about 5 to about 99 weight percent, and more preferably from about 10 to about 99 weight percent, or more preferably from about 40 to about 90 weight percent, or more preferably from about 50 to about 80 weight percent, or more preferably from about 60 to about 80 weight percent.

The monomethyl ester base stock component can also be present as a minor co-base stock in the lubricating oils of this disclosure. Accordingly, the monoester co-base stock component of the present lubricating oils will typically be present from 1 to 50 weight, or more preferably from 5 to 50 percent, or more preferably from 10 to 40 percent, or more preferably from 20 to 30 percent.

#### Other Additives

The formulated lubricating oil useful in the present disclosure may additionally contain one or more of the other commonly used lubricating oil performance additives including but not limited to dispersants, other detergents, corrosion inhibitors, rust inhibitors, metal deactivators, other anti-wear agents and/or extreme pressure additives, anti-seizure agents, wax modifiers, viscosity index improvers, viscosity modifiers, fluid-loss additives, seal compatibility agents, other friction modifiers, lubricity agents, anti-staining agents, chromophoric agents, defoamants, demulsifiers, emulsifiers, densifiers, wetting agents, gelling agents, tackiness agents, colorants, and others. For a review of many commonly used additives, see Klammann in Lubricants and Related Products. Verlag Chemie. Deerfield Beach, Fla.; ISBN 0-89573-177-0. Reference is also made to "Lubricant Additives Chemistry and Applications" edited by Leslie R. Rudnick, Marcel Dekker, Inc. New York, 2003 ISBN: 0-8247-0857-1.

All of the additives described below can be used alone or in combination. The total treat rates for the additives can range from 1 to 30 percent, or more preferably from 2 to 25 percent, or more preferably from 3 to 20 percent, or more

## 16

preferably from 4 to 15 percent, or more preferably from 5 to 10 percent. Particularly preferred compositions have additive levels between and 20 percent.

The types and quantities of performance additives used in combination with the instant disclosure in lubricant compositions are not limited by the examples shown herein as illustrations.

#### Viscosity Improvers

Viscosity improvers (also known as Viscosity Index modifiers, and VI improvers) increase the viscosity of the oil composition at elevated temperatures which increases film thickness, while having limited effect on viscosity at low temperatures.

Suitable viscosity improvers include high molecular weight hydrocarbons, polyesters and viscosity index improver dispersants that function as both a viscosity index improver and a dispersant. Typical molecular weights of these polymers are between about 10,000 to 1,000,000, more typically about 20,000 to 500,000, and even more typically between about 50,000 and 200,000.

Examples of suitable viscosity improvers are polymers and copolymers of methacrylate, butadiene, olefins, or alkylated styrenes. Polyisobutylene is a commonly used viscosity index improver. Another suitable viscosity index improver is polymethacrylate (copolymers of various chain length alkyl methacrylates, for example), some formulations of which also serve as pour point depressants. Other suitable viscosity index improvers include copolymers of ethylene and propylene, hydrogenated block copolymers of styrene and isoprene, and polyacrylates (copolymers of various chain length acrylates, for example). Specific examples include styrene-isoprene or styrene-butadiene based polymers of 50,000 to 200,000 molecular weight.

The amount of viscosity modifier may range from zero to 8 wt %, preferably zero to 4 wt %, more preferably zero to 2 wt % based on active ingredient and depending on the specific viscosity modifier used.

#### Antioxidants

Typical anti-oxidant include phenolic anti-oxidants, aminic anti-oxidants and oil-soluble copper complexes.

The phenolic antioxidants include sulfurized and non-sulfurized phenolic antioxidants. The terms "phenolic type" or "phenolic antioxidant" used herein includes compounds having one or more than one hydroxyl group bound to an aromatic ring which may itself be mononuclear, e.g., benzyl, or poly-nuclear, e.g., naphthyl and spiro aromatic compounds. Thus "phenol type" includes phenol per se, catechol, resorcinol, hydroquinone, naphthol, etc., as well as alkyl or alkenyl and sulfurized alkyl or alkenyl derivatives thereof, and bisphenol type compounds including such bisphenol compounds linked by alkylene bridges sulfuric bridges or oxygen bridges. Alkyl phenols include mono- and poly-alkyl or alkenyl phenols, the alkyl or alkenyl group containing from about 3-100 carbons, preferably 4 to 50 carbons and sulfurized derivatives thereof, the number of alkyl or alkenyl groups present in the aromatic ring ranging from 1 to up to the available unsatisfied valences of the aromatic ring remaining after counting the number of hydroxyl groups bound to the aromatic ring.

Generally, therefore, the phenolic anti-oxidant may be represented by the general formula:



where Ar is selected from the group consisting of:



wherein R is a C<sub>3</sub>-C<sub>100</sub> alkyl or alkenyl group, a sulfur substituted alkyl or alkenyl group, preferably a C<sub>4</sub>-C<sub>50</sub> alkyl or alkenyl group or sulfur substituted alkyl or alkenyl group, more preferably C<sub>3</sub>-C<sub>100</sub> alkyl or sulfur substituted alkyl group, most preferably a C<sub>4</sub>-C<sub>50</sub> alkyl group, R<sup>G</sup> is a C<sub>1</sub>-C<sub>100</sub> alkylene or sulfur substituted alkylene group, preferably a C<sub>2</sub>-C<sub>50</sub> alkylene or sulfur substituted alkylene group, more preferably a C<sub>2</sub>-C<sub>2</sub> alkylene or sulfur substituted alkylene group, y is at least 1 to up to the available valences of Ar, x ranges from 0 to up to the available valences of Ar-y, z ranges from 1 to 10, n ranges from 0 to 20, and m is 0 to 4 and p is 0 or 1, preferably y ranges from 1 to 3, x ranges from 0 to 3, z ranges from 1 to 4 and n ranges from 0 to 5, and p is 0.

Preferred phenolic anti-oxidant compounds are the hindered phenolics and phenolic esters which contain a sterically hindered hydroxyl group, and these include those derivatives of dihydroxy aryl compounds in which the hydroxyl groups are in the o- or p-position to each other. Typical phenolic anti-oxidants include the hindered phenols substituted with C<sub>1</sub>+ alkyl groups and the alkylene coupled derivatives of these hindered phenols. Examples of phenolic materials of this type 2-t-butyl-4-heptyl phenol; 2-t-butyl-4-octyl phenol; 2-t-butyl-4-dodecyl phenol; 2,6-di-t-butyl-4-heptyl phenol; 2,6-di-t-butyl-4-dodecyl phenol; 2-methyl-6-t-butyl-4-heptyl phenol; 2-methyl-6-t-butyl-4-dodecyl phenol; 2,6-di-t-butyl-4 methyl phenol; 2,6-di-t-butyl-4-ethyl phenol; and 2,6-di-t-butyl 4 alkoxy phenol; and



5 Phenolic type anti-oxidants are well known in the lubricating industry and commercial examples such as Ethanox® 4710, Irganox® 1076, Irganox® L1035, Irganox® 1010, Irganox® L109, Irganox® L118, Irganox® L135 and the like are familiar to those skilled in the art. The above is 10 presented only by way of exemplification, not limitation on the type of phenolic anti-oxidants which can be used.

15 The phenolic anti-oxidant can be employed in an amount in the range of about 0.1 to 3 wt %, preferably about 1 to 3 20 wt %, more preferably 1.5 to 3 wt % on an active ingredient basis.

25 Aromatic amine anti-oxidants include phenyl- $\alpha$ -naphthyl amine which is described by the following molecular structure:



30 35 wherein R<sup>Z</sup> is hydrogen or a C<sub>1</sub> to C<sub>14</sub> linear or C<sub>3</sub> to C<sub>14</sub> branched alkyl group, preferably C<sub>1</sub> to C<sub>10</sub> linear or C<sub>3</sub> to C<sub>10</sub> branched alkyl group, more preferably linear or branched C<sub>6</sub> to C<sub>5</sub> and n is an integer ranging from 1 to 5 preferably 1. A particular example is Irganox L06.

40 Other aromatic amine anti-oxidants include other alkylated and non-alkylated aromatic amines such as aromatic monoamines of the formula R<sup>8</sup>R<sup>9</sup>R<sup>10</sup>N where R<sup>8</sup> is an aliphatic, aromatic or substituted aromatic group, R<sup>9</sup> is an aromatic or a substituted aromatic group, and R<sup>10</sup> is H, alkyl, 45 aryl or R<sup>11</sup>S(O)<sub>x</sub>R<sup>12</sup> where R<sup>11</sup> is an alkylene, alkenylene, or aralkylene group, R<sup>12</sup> is a higher alkyl group, or an alkenyl, aryl, or alkaryl group, and x is 0, 1 or 2. The aliphatic group R<sup>8</sup> may contain from 1 to about 20 carbon atoms, and 50 preferably contains from about 6 to 12 carbon atoms. The aliphatic group is a saturated aliphatic group. Preferably, both R<sup>8</sup> and R<sup>9</sup> are aromatic or substituted aromatic groups, and the aromatic group may be a fused ring aromatic group such as naphthyl. Aromatic groups R<sup>8</sup> and R<sup>9</sup> may be joined together with other groups such as S.

55 Typical aromatic amines anti-oxidants have alkyl substituent groups of at least about 6 carbon atoms. Examples of aliphatic groups include hexyl, heptyl, octyl, nonyl, and decyl. Generally, the aliphatic groups will not contain more than about 14 carbon atoms. The general types of such other 60 additional amine anti-oxidants which may be present include diphenylamines, phenothiazines, imidodibenzyls and diphenyl phenylene diamines. Mixtures of two or more of such other additional aromatic amines may also be present. Polymeric amine antioxidants can also be used.

65 Another class of anti-oxidant used in lubricating oil compositions and which may also be present are oil-soluble copper compounds. Any oil-soluble suitable copper com-

pound may be blended into the lubricating oil. Examples of suitable copper antioxidants include copper dihydrocarbyl thio- or dithio-phosphates and copper salts of carboxylic acid (naturally occurring or synthetic). Other suitable copper salts include copper dithiacarbamates, sulphonates, phenates, and acetylacetones. Basic, neutral, or acidic copper Cu(I) and or Cu(II) salts derived from alkenyl succinic acids or anhydrides are known to be particularly useful.

Such antioxidants may be used individually or as mixtures of one or more types of antioxidants, the total amount employed being an amount of about 0.50 to 5 wt %, preferably about 0.75 to 3 wt % (on an as-received basis). Detergents

In addition to the alkali or alkaline earth metal salicylate detergent which is an essential component in the present disclosure, other detergents may also be present. While such other detergents can be present, it is preferred that the amount employed be such as to not interfere with the synergistic effect attributable to the presence of the salicylate. Therefore, most preferably such other detergents are not employed.

If such additional detergents are present, they can include alkali and alkaline earth metal phenates, sulfonates, carboxylates, phosphonates and mixtures thereof. These supplemental detergents can have total base number (TBN) ranging from neutral to highly overbased, i.e. TBN of 0 to over 500, preferably 2 to 400, more preferably 5 to 300, and they can be present either individually or in combination with each other in an amount in the range of from 0 to 10 wt %, preferably 0.5 to 5 wt % (active ingredient) based on the total weight of the formulated lubricating oil. As previously stated, however, it is preferred that such other detergent not be present in the formulation.

Such additional other detergents include by way of example and not limitation calcium phenates, calcium sulfonates, magnesium phenates, magnesium sulfonates and other related components (including borated detergents).

#### Dispersants

During engine operation, oil-insoluble oxidation byproducts are produced. Dispersants help keep these byproducts in solution, thus diminishing their deposition on metal surfaces. Dispersants may be ashless or ash-forming in nature. Preferably, the dispersant is ashless. So called ashless dispersants are organic materials that form substantially no ash upon combustion. For example, non-metal-containing or borated metal-free dispersants are considered ashless. In contrast, metal-containing detergents discussed above form ash upon combustion.

Suitable dispersants typically contain a polar group attached to a relatively high molecular weight hydrocarbon chain. The polar group typically contains at least one element of nitrogen, oxygen, or phosphorus. Typical hydrocarbon chains contain 50 to 400 carbon atoms.

A particularly useful class of dispersants are the alkenylsuccinic derivatives, typically produced by the reaction of a long chain substituted alkenyl succinic compound, usually a substituted succinic anhydride, with a polyhydroxy or polyamino compound. The long chain group constituting the oleophilic portion of the molecule which confers solubility in the oil, is normally a polyisobutylene group. Many examples of this type of dispersant are well known commercially and in the literature. Exemplary patents describing such dispersants are U.S. Pat. Nos. 3,172,892; 3,219,666; 3,316,177 and 4,234,435. Other types of dispersants are described in U.S. Pat. Nos. 3,036,003; and 5,705,458.

Hydrocarbyl-substituted succinic acid compounds are popular dispersants. In particular, succinimide, succinate

esters, or succinate ester amides prepared by the reaction of a hydrocarbon-substituted succinic acid compound preferably having at least 50 carbon atoms in the hydrocarbon substituent, with at least one equivalent of an alkylene amine are particularly useful.

Succinimides are formed by the condensation reaction between alkenyl succinic anhydrides and amines. Molar ratios can vary depending on the amine or polyamine. For example, the molar ratio of alkenyl succinic anhydride to TEPA can vary from about 1:1 to about 5:1.

Succinate esters are formed by the condensation reaction between alkenyl succinic anhydrides and alcohols or polyols. Molar ratios can vary depending on the alcohol or polyol used. For example, the condensation product of an alkenyl succinic anhydride and pentaerythritol is a useful dispersant.

Succinate ester amides are formed by condensation reaction between alkenyl succinic anhydrides and alkanol amines. For example, suitable alkanol amines include ethoxylated polyalkylpolyamines, propoxylated polyalkylpolyamines and polyalkenylpolyamines such as polyethylene polyamines. One example is propoxylated hexamethylenediamine.

The molecular weight of the alkenyl succinic anhydrides will typically range between 800 and 2,500. The above products can be post-reacted with various reagents such as sulfur, oxygen, formaldehyde, carboxylic acids such as oleic acid, and boron compounds such as borate esters or highly borated dispersants. The dispersants can be borated with from about 0.1 to about moles of boron per mole of dispersant reaction product.

Mannich base dispersants are made from the reaction of alkylphenols, formaldehyde, and amines. Process aids and catalysts, such as oleic acid and sulfonic acids, can also be part of the reaction mixture. Molecular weights of the alkylphenols range from 800 to 2,500.

Typical high molecular weight aliphatic acid modified Mannich condensation products can be prepared from high molecular weight alkyl-substituted hydroxyaromatics or HN(R)<sub>2</sub> group-containing reactants.

Examples of high molecular weight alkyl-substituted hydroxyaromatic compounds are polypropylphenol, polybutylphenol, and other polyalkylphenols. These polyalkylphenols can be obtained by the alkylation, in the presence of an alkylating catalyst, such as BF<sub>3</sub>, of phenol with high molecular weight polypropylene, polybutylene, and other polyalkylene compounds to give alkyl substituents on the benzene ring of phenol having an average 600-100,000 molecular weight.

Examples of HN(R)<sub>2</sub> group-containing reactants are alkylene polyamines, principally polyethylene polyamines. Other representative organic compounds containing at least one HN(R)<sub>2</sub> group suitable for use in the preparation of Mannich condensation products are well known and include the mono- and di-amino alkanes and their substituted analogs, e.g., ethylamine and diethanol amine; aromatic diamines, e.g., phenylene diamine, diamino naphthalenes; heterocyclic amines, e.g., morpholine, pyrrole, pyrrolidine, imidazole, imidazolidine, and piperidine; melamine and their substituted analogs.

Examples of alkylene polyamine reactants include ethylenediamine, diethylene triamine, triethylene tetraamine, tetraethylene pentaamine, pentaethylene hexamine, hexaethylene heptaamine, heptaethylene octaamine, octaethylene nonaamine, nonaethylene decamine, and decathylenediamine and mixture of such amines having nitrogen contents corresponding to the alkylene polyamines, in the formula H<sub>2</sub>N—(Z—NH—)<sub>n</sub>H, mentioned before, Z is a divalent

ethylene and n is 1 to 10 of the foregoing formula. Corresponding propylene polyamines such as propylene diamine and di-, tri-, tetra-, pentapropylene tri-, tetra-, penta- and hexaamines are also suitable reactants. The alkylene polyamines are usually obtained by the reaction of ammonia and dihalo alkanes, such as dichloro alkanes. Thus the alkylene polyamines obtained from the reaction of 2 to 11 moles of ammonia with 1 to 10 moles of dichloroalkanes having 2 to 6 carbon atoms and the chlorines on different carbons are suitable alkylene polyamine reactants.

Aldehyde reactants useful in the preparation of the high molecular products useful in this disclosure include the aliphatic aldehydes such as formaldehyde (also as paraformaldehyde and formalin), acetaldehyde and aldol ( $\beta$ -hydroxybutyraldehyde). Formaldehyde or a formaldehyde-yielding reactant is preferred.

Preferred dispersants include borated and non-borated succinimides, including those derivatives from mono-succinimides, bis-succinimides, and/or mixtures of mono- and bis-succinimides, wherein the hydrocarbyl succinimide is derived from a hydrocarbylene group such as polyisobutylene having a Mn of from about 500 to about 5000 or a mixture of such hydrocarbylene groups. Other preferred dispersants include succinic acid-esters and amides, alkyl-phenol-polyamine-coupled Mannich adducts, their capped derivatives, and other related components. Such additives may be used in an amount of about 0.1 to 20 wt %, preferably about 0.1 to 8 wt %, more preferably about 1 to 6 wt % (on an as-received basis) based on the weight of the total lubricant.

#### Pour Point Depressants

Conventional pour point depressants (also known as lube oil flow improvers) may also be present. Pour point depressant may be added to lower the minimum temperature at which the fluid will flow or can be poured. Examples of suitable pour point depressants include alkylated naphthalenes polymethacrylates, polyacrylates, polyarylamides, condensation products of haloparaffin waxes and aromatic compounds, vinyl carboxylate polymers, and terpolymers of dialkylfumarates, vinyl esters of fatty acids and allyl vinyl ethers. Such additives may be used in amount of about 0.0 to 0.5 wt %, preferably about 0 to 0.3 wt %, more preferably about 0.001 to 0.1 wt % on an as-received basis.

#### Corrosion Inhibitors/Metal Deactivators

Corrosion inhibitors are used to reduce the degradation of metallic parts that are in contact with the lubricating oil composition. Suitable corrosion inhibitors include aryl thiazines, alkyl substituted dimercapto thiodiazoles thiadiazoles and mixtures thereof. Such additives may be used in an amount of about 0.01 to 5 wt % preferably about 0.01 to 1.5 wt %, more preferably about 0.01 to 0.2 wt %, still more preferably about 0.01 to 0.1 wt % (on an as-received basis) based on the total weight of the lubricating oil composition.

#### Seal Compatibility Additives

Seal compatibility agents help to swell elastomeric seals by causing a chemical reaction in the fluid or physical change in the elastomer. Suitable seal compatibility agents for lubricating oils include organic phosphates, aromatic esters, aromatic hydrocarbons, esters (butylbenzyl phthalate, for example), and polybutenyl succinic anhydride and sulfolane-type seal swell agents such as Lubrizol 730-type seal swell additives. Such additives may be used in an amount of about 0.01 to 3 wt %, preferably about 0.01 to 2 wt % on an as-received basis.

#### Anti-Foam Agents

Anti-foam agents may advantageously be added to lubricant compositions. These agents retard the formation of

stable foams. Silicones and organic polymers are typical anti-foam agents. For example, polysiloxanes, such as silicon oil or polydimethyl siloxane, provide antifoam properties. Anti-foam agents are commercially available and may be used in conventional minor amounts along with other additives such as demulsifiers; usually the amount of these additives combined is less than 1 percent, preferably 0.001 to about 0.5 wt %, more preferably about 0.001 to about 0.2 wt %, still more preferably about 0.0001 to 0.15 wt % (on an as-received basis) based on the total weight of the lubricating oil composition.

#### Inhibitors and Antirust Additives

Anti-rust additives (or corrosion inhibitors) are additives that protect lubricated metal surfaces against chemical attack by water or other contaminants. One type of anti-rust additive is a polar compound that wets the metal surface preferentially, protecting it with a film of oil. Another type of anti-rust additive absorbs water by incorporating it in a water-in-oil emulsion so that only the oil touches the surface. Yet another type of anti-rust additive chemically adheres to the metal to produce a non-reactive surface. Examples of suitable additives include zinc dithiophosphates, metal phenolates, basic metal sulfonates, fatty acids and amines. Such additives may be used in an amount of about 0.01 to 5 wt %, preferably about 0.01 to 1.5 wt % on an as-received basis.

In addition to the ZDDP anti-wear additives which are essential components of the present disclosure, other anti-wear additives can be present, including zinc dithiocarbamates, molybdenum dialkyldithiophosphates, molybdenum dithiocarbamates, other organo molybdenum-nitrogen complexes, sulfurized olefins, etc.

The term "organo molybdenum-nitrogen complexes" embraces the organo molybdenum-nitrogen complexes described in U.S. Pat. No. 4,889,647. The complexes are reaction products of a fatty oil, dithanolamine and a molybdenum source. Specific chemical structures have not been assigned to the complexes. U.S. Pat. No. 4,889,647 reports an infrared spectrum for a typical reaction product of that disclosure: the spectrum identifies an ester carbonyl band at  $1740\text{ cm}^{-1}$  and an amide carbonyl band at  $1620\text{ cm}^{-1}$ . The fatty oils are glyceryl esters of higher fatty acids containing at least 12 carbon atoms up to 22 carbon atoms or more. The molybdenum source is an oxygen-containing compound such as ammonium molybdates, molybdenum oxides and mixtures.

Other organo molybdenum complexes which can be used in the present disclosure are tri-nuclear molybdenum-sulfur compounds described in EP 1 040 115 and WO 99/31113 and the molybdenum complexes described in U.S. Pat. No. 4,978,464.

#### Performance and Uses

The lubricant compositions of this disclosure give advantaged performance in the lubrication of internal combustion engines, power trains, drivelines, transmissions, gears, gear trains, gear sets, compressors, pumps, hydraulic systems, bearings, bushings, turbines, and the like.

Also, the lubricant compositions of this disclosure give advantaged friction, wear, and other lubricant performances in the lubrication of mechanical components, which comprise, for example, pistons, piston rings, cylinder liners, cylinders, cams, tappets, lifters, bearings (journal, roller, tapered, needle, ball, and the like), gears, valves, and the like.

Further, the lubricant compositions of this disclosure give advantaged friction, wear, and other lubricant performances under a range of lubrication contact pressures, from 1 MPas

to greater than 10 GPas, preferably greater than 10 MPas, more preferably greater than 100 MPas, even more preferably greater than 300 MPas. Under certain circumstances, the instant disclosure gives advantaged wear and friction performance at greater than 0.5 GPas, often at greater than 1 GPas, sometimes greater than 2 GPas, under selected circumstances greater than 5 GPas.

Yet further, the lubricant compositions of this disclosure give advantaged friction, wear, and other lubricant performances when used in combination with lubricated surfaces comprising: metals, metal alloys, non-metals, non-metal alloys, mixed carbon-metal composites and alloys, mixed carbon-nonmetal composites and alloys, ferrous metals, ferrous composites and alloys, non-ferrous metals, non-ferrous composites and alloys, titanium, titanium composites and alloys, aluminum, aluminum composites and alloys, magnesium, magnesium composites and alloys, ion-implanted metals and alloys, plasma modified surfaces; surface modified materials; coatings; mono-layer, multi-layer, and gradient layered coatings; honed surfaces; polished surfaces; etched surfaces; textured surfaces; micro and nano structures on textured surfaces; super-finished surfaces; diamond-like carbon (DLC), DLC with high-hydrogen content, DLC with moderate hydrogen content. DLC with low-hydrogen content. DLC with zero hydrogen content. DLC composites, DLC-metal compositions and composites, DLC-nonmetal compositions and composites; glasses, metallic glasses; ceramics, cermets, ceramic oxides, ceramic nitrides, FeN, CrN, ceramic carbides, mixed ceramic compositions, and the like; polymers, plastics, thermoplastic polymers, engineered polymers, polymer blends, polymer alloys, polymer composites; elastomers; materials compositions and composites containing dry lubricants, comprising for example graphite, carbon, molybdenum, molybdenum disulfide, polytetrafluoroethylene, polyperfluoropropylene, polyperfluoroalkylethers, and the like.

The viscometric properties of the lubricants of this disclosure can be measured according to standard practices. A low viscosity can be advantageous for lubricants in modern equipment. A low high temperature high shear (HTHS) viscosity, in accordance with ASTM D4683, can indicate performance of a lubricant in a modern engine. In particular, the lubricants of this disclosure can have an HTHS of less than 2.0 cP, or more preferably less than 1.9 cP, or more preferably less than 1.8 cP, or more preferably less than 1.7 cP.

The lubricants of this disclosure can have lower volatility, as determined by the Noack volatility test ASTM D5800, or as predicted by a TGA test that simulates the Noack vola-

The lubricants of this disclosure can have lower deposition tendency, as determined by the TEOST 33C deposition test ASTM D6335. In particular, the lubricants of this disclosure can have a TEOST 33C of less than 30 mg, or more preferably less than 20 mg, or more preferably less than 15 mg.

The lubricants of this disclosure can have reduced traction as determined by the MTM (Mini Traction Machine) traction test. Traction is most easily assessed by comparison to a reference fluid, in this case a suitable reference fluid is an engine oil formulated with commercial dioctyl adipate ester such as Esterex™ A32. Accordingly, the lubricants of this disclosure can have an MTM traction reduction of 5% versus a reference, or more preferably a reduction of 10% versus a reference, or more preferably a reduction of 20% versus a reference, or more preferably a reduction of 30% versus a reference, or more preferably a reduction of 40% versus a reference.

In the above detailed description, the specific embodiments of this disclosure have been described in connection with its preferred embodiments. However, to the extent that the above description is specific to a particular embodiment or a particular use of this disclosure, this is intended to be illustrative only and merely provides a concise description of the exemplary embodiments. Accordingly, the disclosure is not limited to the specific embodiments described above, but rather, the disclosure includes all alternatives, modifications, and equivalents falling within the true scope of the appended claims. Various modifications and variations of this disclosure will be obvious to a worker skilled in the art and it is to be understood that such modifications and variations are to be included within the purview of this application and the spirit and scope of the claims.

## EXAMPLES

### Examples 1 to 3

#### Preparation of Near Linear, Mono-Esters from NEODOL 67 Alcohols

To a round bottom flask equipped with a Dean-Stark trap was added NEODOL 67 alcohol (branched mono-methyl C<sub>16</sub> to C<sub>17</sub> alcohol), n-carboxylic acid (5-25% mole excess) (Example 1—linear hexanoic acid, Example 2—linear octanoic acid and Example 3—linear decanoic acid), titanium (IV) isopropoxide (0.02 mol %), toluene (5-10 wt. %), and activated carbon (0.2 wt. %). The mixture was heated to reflux at 180° C. until the NEODOL 67 was consumed per the reaction scheme below.



tility. In particular, the lubricants of this disclosure can have a Noack between 1% and 50%, or more preferably between 10% and 50%, or more preferably between 15% and 40%, or more preferably between 20% and 30%. Particularly preferred compositions have a Noack between 15% and 30%.

Toluene was removed by distillation at 180° C. Excess acid was stripped under vacuum at 180° C. The distillation pot bottoms were cooled to 70° C. and treated with lime (1 wt. %) and water (1 wt. %) with stirring for 20 minutes. The water was removed under vacuum distillation at 90° C. The distillation pot bottoms was filtered to remove carbon and lime. The monomethyl ester basestock was collected as the

filtrate in greater than 60% isolated yield. Three alternative monomethyl ester basestocks were produced as indicated by Examples 1 to 3 or Fluids 1 to 3 below.

Example 1 or Fluid 1



Example 2 or Fluid 2



Example 3 or Fluid 3



For Examples 1 to 3 above, the methyl group or branch is located at the eighth carbon of the linear chain. However, the methyl branch may vary anywhere from the second carbon to the fifteenth carbon of the linear chain. More particularly, the methyl branch may occur at the second, or third, or fourth, or fifth, or sixth, or seventh, or eighth, or ninth, or tenth, or eleventh, or twelfth, or thirteenth, or fourteenth, or fifteenth carbon of the linear chain.

Lube Properties

The lube properties of the products of Examples 1-3 were evaluated as Group V basestocks and the results are shown in Table 4 below. The kinematic viscosity (K<sub>v</sub>) of the liquid product was measured using ASTM D445 or D7042, and reported at temperatures of 100° C. (K<sub>v</sub> at 100° C.) or 40° C. (K<sub>v</sub> at 40° C.). The viscosity index (VI) was measured according to ASTM D2270 using the measured kinematic viscosities for each product. Noack volatility was determined by ASTM D5800. Pour point was determined by ASTM D97.

TABLE 4

| Fluid | Ester                       | K <sub>v</sub> <sub>100</sub><br>cSt | K <sub>v</sub> <sub>40</sub><br>cSt | VI  | Noack | Pour<br>Point, ° C. |
|-------|-----------------------------|--------------------------------------|-------------------------------------|-----|-------|---------------------|
| 1     | nC <sub>6</sub> -NEODOL 67  | 2.39                                 | 7.44                                | 155 | 41.2  | -39                 |
| 2     | nC <sub>8</sub> -NEODOL 67  | 2.73                                 | 9.01                                | 157 | 24.4  | -21                 |
| 3     | nC <sub>10</sub> -NEODOL 67 | 3.17                                 | 11.0                                | 164 | 14.8  | -15                 |

Table 4 clearly shows that the monomethyl ester base stock examples of this disclosure (Examples 1-3) all have desirable viscosity-volatility properties. That is a combination of low viscosity and low volatility as measured by Noack. Surprisingly, the monomethyl ester base stock examples also have outstanding cold flow properties as measured by a high Viscosity Index and a low pour point.

30 PCT and EP Clauses:

1. A lubricating oil base stock comprising one or more compounds represented by the formula



40 wherein R<sub>1</sub> is a monomethyl branched C<sub>15</sub> to C<sub>19</sub> alkyl group and R<sub>2</sub> is an unsubstituted C<sub>2</sub> to C<sub>30</sub> linear alkyl group, and

45 wherein said base stock has a viscosity (K<sub>v</sub><sub>100</sub>) from about 1 cSt to about 10 cSt at 100° C. as determined by ASTM D445, a viscosity index (VI) from about -100 to about 300 as determined by ASTM D2270, a pour points from about 0° C. to about -50° C. as determined by ASTM D97, and a Noack volatility of no greater than 50 percent as determined by ASTM D5800.

50 2. The lubricating oil base stock of clause 1 wherein R<sub>1</sub> is a monomethyl branched C<sub>16</sub> to C<sub>17</sub> alkyl group.

3. The lubricating oil base stock of clauses 1-2 wherein R<sub>1</sub> is a monomethyl branched C<sub>1</sub> to C<sub>1</sub> alkyl group.

4. The lubricating oil base stock of clauses 1-3 wherein R<sub>1</sub> is a monomethyl branched C<sub>17</sub> alkyl group.

5. The lubricating oil base stock of clauses 1-4 wherein R<sub>2</sub> is an unsubstituted C<sub>5</sub> to C<sub>9</sub> linear alkyl group.

6. The lubricating oil base stock of clauses 1-5 wherein the monomethyl branch is positioned from the second carbon to the fifteenth carbon of the alkyl group.

60 7. The lubricating oil base stock of clauses 1-6 wherein the monomethyl branch is positioned at the eighth carbon of the alkyl group.

8. The lubricating oil base stock of clause 1 which is selected from the group consisting of 8-methylpentadecyl hexanoate, 8-methylpentadecyl octanoate, 8-methylpentadecyl decanoate, and combinations thereof.

65 9. The lubricating oil base stock of clauses 1-8 which has a viscosity (K<sub>v</sub><sub>100</sub>) from about 2 cSt to about 8 cSt at 100°

C. as determined by ASTM D445, a viscosity index (VI) from about 25 to about 150 as determined by ASTM D2270, a pour points from about -20° C. to about -50° C. as determined by ASTM D97, and a Noack volatility of no greater than 25 percent as determined by ASTM D5800.

10. The lubricating oil base stock of clauses 1-9 further comprising one or more of a viscosity improver, antioxidant, detergent, dispersant, pour point depressant, corrosion inhibitor, metal deactivator, seal compatibility additive, anti-foam agent, inhibitor, and anti-rust additive.

11. A lubricating oil base stock comprising one or more compounds represented by the formula



wherein  $\text{R}_1$  is a monomethyl branched  $\text{C}_{15}$  to  $\text{C}_{19}$  alkyl group and  $\text{R}_2$  is selected from the group consisting of a substituted or unsubstituted  $\text{C}_4$ - $\text{C}_{30}$  aryl group, a substituted or unsubstituted  $\text{C}_4$ - $\text{C}_{30}$  heteroaryl group, a  $\text{C}_5$ - $\text{C}_{30}$  arylalkyl group and a substituted or unsubstituted  $\text{C}_1$ - $\text{C}_{30}$  alkoxy group, and wherein said base stock has a viscosity ( $\text{Kv}_{100}$ ) from about 1 cSt to about 10 cSt at 100° C. as determined by ASTM D445, a viscosity index (VI) from about -100 to about 300 as determined by ASTM D2270, a pour points from about 0° C. to about -50° C. as determined by ASTM D97, and a Noack volatility of no greater than 50 percent as determined by ASTM D5800

wherein said one or more compounds are produced by a process comprising reacting a monomethyl substituted  $\text{C}_{15}$  to  $\text{C}_{19}$  linear alcohol with a carboxylic acid, an aromatic alkanoic acid, or a glycol ether acid, optionally in the presence of a catalyst and a solvent, under reaction conditions sufficient to produce said one or more compounds.

12. The lubricating oil base stock of clause 11 wherein  $\text{R}_1$  is a monomethyl branched  $\text{C}_{16}$  to  $\text{C}_{17}$  alkyl group.

13. The lubricating oil base stock of clauses 11-12 wherein the carboxylic acid is selected from the group consisting of isobutyric acid, 2-ethylhexanoic acid, 2-butylhexanoic acid, 2-butyloctanoic acid, 2-hexyldecanoic acid, 2-heptylundecanoic acid, 2-octyldecanoic acid, 2-decyldodecanoic acid, isotridecanoic acid and combinations thereof.

14. The lubricating oil base stock of clauses 11-12 wherein the aromatic alkanoic acid is selected from the group consisting of benzoic acid, phenylacetic acid, phenylpropionic acid, phenylbutyric acid, methoxyphenylacetic acid, tolylacetic acid, nitrophenylacetic acid, xylylacetic acid, tolylpropionic acid, xylylpropionic acid, methoxyphenylpropionic acid, methoxyphenylbutyric acid, nitrophenylpropionic acid, nitrophenylbutyric acid, xylylbutyric acid, tolylbutyric acid and combinations thereof.

15. The lubricating oil base stock of clauses 11-12 wherein the glycol ether acid is selected from the group consisting of methoxyacetic acid, methoxypropionic acid, methoxyethoxyacetic acid, methoxyethoxyethoxyacetic acid, ethoxyacetic acid, ethoxyethoxyacetic acid, ethoxyethoxyacetic acid, propoxyacetic acid, propoxyethoxyacetic acid, butoxyethoxyacetic acid, butoxyethoxyethoxyacetic acid, propoxybenzoic acid and combinations thereof.

16. The lubricating oil base stock of clauses 11-15 further comprising one or more of a viscosity improver, antioxidant, detergent, dispersant, pour point depressant, corrosion

inhibitor, metal deactivator, seal compatibility additive, anti-foam agent inhibitor, anti-rust additive and combinations thereof.

All patents and patent applications, test procedures (such as ASTM methods, UL methods, and the like), and other documents cited herein are fully incorporated by reference to the extent such disclosure is not inconsistent with this disclosure and for all jurisdictions in which such incorporation is permitted.

10. When numerical lower limits and numerical upper limits are listed herein, ranges from any lower limit to any upper limit are contemplated. While the illustrative embodiments of the disclosure have been described with particularity, it will be understood that various other modifications will be apparent to and can be readily made by those skilled in the art without departing from the spirit and scope of the disclosure. Accordingly, it is not intended that the scope of the claims appended hereto be limited to the examples and descriptions set forth herein but rather that the claims be construed as encompassing all the features of patentable novelty which reside in the present disclosure, including all features which would be treated as equivalents thereof by those skilled in the art to which the disclosure pertains.

The present disclosure has been described above with reference to numerous embodiments and specific examples. Many variations will suggest themselves to those skilled in this art in light of the above detailed description. All such obvious variations are within the full intended scope of the appended claims.

30. The invention claimed is:

1. A monomethyl ester composition comprising one or more compounds represented by the formula:



wherein  $\text{R}_1$  is a monomethyl branched  $\text{C}_{15}$  to  $\text{C}_{19}$  alkyl group and  $\text{R}_2$  is an unsubstituted  $\text{C}_2$  to  $\text{C}_{30}$  linear alkyl group, and wherein said composition has a viscosity ( $\text{Kv}_{100}$ ) from about 1 cSt to about 10 cSt at 100° C. as determined by ASTM D445, a viscosity index (VI) from about -100 to about 300 as determined by ASTM D2270, a pour point from about 0° C. to about -50° C. as determined by ASTM D97, and a Noack volatility of no greater than 50 percent as determined by ASTM D5800.

2. The composition of claim 1 wherein  $\text{R}_1$  is a monomethyl branched  $\text{C}_{16}$  to  $\text{C}_{17}$  alkyl group.

3. The composition of claim 1 wherein  $\text{R}_1$  is a monomethyl branched  $\text{C}_{16}$  alkyl group.

4. The composition of claim 1 wherein  $\text{R}_1$  is a monomethyl branched  $\text{C}_{17}$  alkyl group.

5. The composition of claim 1 wherein  $\text{R}_2$  is an unsubstituted  $\text{C}_5$  to  $\text{C}_9$  linear alkyl group.

6. The composition of claim 2 wherein the monomethyl branch is positioned from the second carbon to the fifteenth carbon of the alkyl group.

7. The composition of claim 2 wherein the monomethyl branch is positioned at the eighth carbon of the alkyl group.

8. The composition of claim 1 which is selected from the group consisting of 8-methylpentadecyl hexanoate, 8-methylpentadecyl octanoate, 8-methylpentadecyl decanoate, and combinations thereof.

9. The composition of claim 1 which has a viscosity ( $\text{Kv}_{100}$ ) from about 2 cSt to about 8 cSt at 100° C. as

29

determined by ASTM D445, a viscosity index (VI) from about 25 to about 150 as determined by ASTM D2270, a pour points from about  $-20^{\circ}\text{C}$ . to about  $-50^{\circ}\text{C}$ . as determined by ASTM D97, and a Noack volatility of no greater than 25 percent as determined by ASTM D5800.

10. A monomethyl ester composition comprising one or more compounds represented by the formula:



wherein  $\text{R}_1$  is a monomethyl branched  $\text{C}_{15}$  to  $\text{C}_{19}$  alkyl group and  $\text{R}_2$  is an unsubstituted  $\text{C}_2$  to  $\text{C}_{30}$  linear alkyl group, and

wherein said composition has a viscosity ( $\text{Kv}_{100}$ ) from about 1 cSt to about 10 cSt at  $100^{\circ}\text{C}$ . as determined by ASTM D445, a viscosity index (VI) from about  $-100$  to about 300 as determined by ASTM D2270, a pour points from about  $0^{\circ}\text{C}$ . to about  $-50^{\circ}\text{C}$ . as determined by ASTM D97, and a Noack volatility of no greater than 50 percent as determined by ASTM D5800; wherein said one or more compounds are produced by a process comprising reacting a monomethyl substituted  $\text{C}_{15}$  to  $\text{C}_{19}$  linear alcohol with an unsubstituted  $\text{C}_2$  to  $\text{C}_{30}$  linear aliphatic acid, optionally in the presence of a catalyst and a solvent, under reaction conditions sufficient to produce said one or more compounds.

11. A lubricating oil base stock comprising one or more compounds represented by the formula



wherein  $\text{R}_1$  is a monomethyl branched  $\text{C}_{15}$  to  $\text{C}_{19}$  alkyl group and  $\text{R}_2$  is an unsubstituted  $\text{C}_2$  to  $\text{C}_{30}$  linear alkyl group, and

wherein said base stock has a viscosity ( $\text{Kv}_{100}$ ) from about 1 cSt to about 10 cSt at  $100^{\circ}\text{C}$ . as determined by ASTM D445, a viscosity index (VI) from about  $-100$  to about 300 as determined by ASTM D2270, a pour points from about  $0^{\circ}\text{C}$ . to about  $-50^{\circ}\text{C}$ . as determined by ASTM D97, and a Noack volatility of no greater than 50 percent as determined by ASTM D5800.

12. The lubricating oil base stock of claim 11 wherein  $\text{R}_1$  is a monomethyl branched  $\text{C}_{16}$  to  $\text{C}_{17}$  alkyl group.

13. The lubricating oil base stock of claim 11 wherein  $\text{R}_1$  is a monomethyl branched  $\text{C}_{16}$  alkyl group.

14. The lubricating oil base stock of claim 11 wherein  $\text{R}_1$  is a monomethyl branched  $\text{C}_{17}$  alkyl group.

15. The lubricating oil base stock of claim 11 wherein  $\text{R}_2$  is an unsubstituted  $\text{C}_5$  to  $\text{C}_9$  linear alkyl group.

16. The lubricating oil base stock of claim 12 wherein the monomethyl branch is positioned from the second carbon to the fifteenth carbon of the alkyl group.

17. The lubricating oil base stock of claim 12 wherein the monomethyl branch is positioned at the eighth carbon of the alkyl group.

18. The lubricating oil base stock of claim 11 which is selected from the group consisting of 8-methylpentadecyl hexanoate, 8-methylpentadecyl octanoate, 8-methylpentadecyl decanoate, and combinations thereof.

19. The lubricating oil base stock of claim 11 which has a viscosity ( $\text{Kv}_{100}$ ) from about 2 cSt to about 8 cSt at  $100^{\circ}\text{C}$ .

30

C. as determined by ASTM D445, a viscosity index (VI) from about 25 to about 150 as determined by ASTM D2270, a pour points from about  $-20^{\circ}\text{C}$ . to about  $-50^{\circ}\text{C}$ . as determined by ASTM D97, and a Noack volatility of no greater than 25 percent as determined by ASTM D5800.

20. The lubricating oil base stock of claim 11 further comprising one or more of a viscosity improver, antioxidant, detergent, dispersant, pour point depressant, corrosion inhibitor, metal deactivator, seal compatibility additive, anti-foam agent, inhibitor, and anti-rust additive.

21. A lubricating oil comprising a lubricating oil base stock component comprising a polyalphaolefin (PAO) or gas-to-liquid (GTL) oil base stock, and a monomethyl ester cobase stock component; wherein said monomethyl ester cobase stock comprises one or more compounds represented by the formula



wherein  $\text{R}_1$  is a monomethyl branched  $\text{C}_{15}$  to  $\text{C}_{19}$  alkyl group and  $\text{R}_2$  is an unsubstituted  $\text{C}_2$  to  $\text{C}_{30}$  linear alkyl group, and

wherein said lubricating oil has a viscosity ( $\text{Kv}_{100}$ ) from about 1 cSt to about 10 cSt at  $100^{\circ}\text{C}$ . as determined by ASTM D445, a viscosity index (VI) from about  $-100$  to about 300 as determined by ASTM D2270, a pour points from about  $0^{\circ}\text{C}$ . to about  $-50^{\circ}\text{C}$ . as determined by ASTM D97, and a Noack volatility of no greater than 50 percent as determined by ASTM D5800.

22. The lubricating oil of claim 21 wherein the lubricating oil base stock is present in an amount from about 1 weight percent to about 99 weight percent, and the monoester cobase stock is present in an amount from about 1 weight percent to about 99 weight percent, based on the total weight of the lubricating oil.

23. The lubricating oil of claim 21 wherein  $\text{R}_1$  is a monomethyl branched  $\text{C}_{16}$  to  $\text{C}_{17}$  alkyl group.

24. The lubricating oil of claim 21 wherein  $\text{R}_1$  is a monomethyl branched  $\text{C}_{16}$  alkyl group.

25. The lubricating oil of claim 21 wherein  $\text{R}_1$  is a monomethyl branched  $\text{C}_{17}$  alkyl group.

26. The lubricating oil of claim 21 wherein  $\text{R}_1$  is an unsubstituted  $\text{C}_5$  to  $\text{C}_9$  linear alkyl group.

27. The lubricating oil of claim 21 which said one or more compounds are selected from the group consisting of 8-methylpentadecyl hexanoate, 8-methylpentadecyl octanoate, 8-methylpentadecyl decanoate, and combinations thereof.

28. The lubricating oil of claim 21 which has a viscosity ( $\text{Kv}_{100}$ ) from about 2 cSt to about 8 cSt at  $100^{\circ}\text{C}$ . as determined by ASTM D445, a viscosity index (VI) from about 25 to about 150 as determined by ASTM D2270, a pour points from about  $-20^{\circ}\text{C}$ . to about  $-50^{\circ}\text{C}$ . as determined by ASTM D97, and a Noack volatility of no greater than 25 percent as determined by ASTM D5800.

29. The lubricating oil of claim 21 further comprising one or more of a viscosity improver, antioxidant, detergent, dispersant, pour point depressant, corrosion inhibitor, metal deactivator, seal compatibility additive, anti-foam agent, inhibitor, and anti-rust additive.

30. A method for improving one or more of cold flow properties, thermal and oxidative stability, solubility and dispersancy of polar additives, deposit control and traction control in a lubricating oil comprising:

31

providing a lubricating oil to an internal combustion engine or a transmission of an automobile engine or truck engine including a lubricating oil base stock component comprising a polyalphaolefin (PAO) or gas-to-liquid (GTL) oil base stock, and a monoester cobase stock component; wherein said monoester cobase stock comprises one or more compounds represented by the formula



wherein  $\text{R}_1$  is a monomethyl branched  $\text{C}_{15}$  to  $\text{C}_1$  alkyl group and  $\text{R}_2$  is an unsubstituted  $\text{C}_2$  to  $\text{C}_{30}$  linear alkyl group, and wherein said lubricating oil has a viscosity ( $\text{Kv}_{100}$ ) from about 1 cSt to about 10 cSt at  $100^\circ \text{C}$ . as determined by ASTM D445, a viscosity index (VI) from about -100 to about 300 as determined by ASTM D2270, a pour points from about  $0^\circ \text{C}$ . to about  $-50^\circ \text{C}$ . as determined by ASTM D97, and a Noack volatility of no greater than 50 percent as determined by ASTM D5800, and using the lubricating oil in the internal combustion engine or the transmission of an automobile engine or truck engine to improve one or more of cold flow properties, thermal and oxidative stability, solubility and dispersancy of polar additives, deposit control and traction control.

31. The method of claim 30 wherein the lubricating oil base stock is present in an amount from about 1 weight

32

percent to about 99 weight percent, and the monoester cobase stock is present in an amount from about 1 weight percent to about 99 weight percent, based on the total weight of the lubricating oil.

5 32. The method of claim 30 wherein  $\text{R}_1$  is a monomethyl branched  $\text{C}_{16}$  to  $\text{C}_{17}$  alkyl group.

33. The method of claim 30 wherein  $\text{R}_1$  is a monomethyl branched  $\text{C}_{16}$  alkyl group.

10 34. The method of claim 30 wherein  $\text{R}_1$  is a monomethyl branched  $\text{C}_{17}$  alkyl group.

35. The method of claim 30 wherein  $\text{R}_2$  is an unsubstituted  $\text{C}_5$  to  $\text{C}_9$  linear alkyl group.

15 36. The method of claim 30 which said one or more compounds are selected from the group consisting of 8-methylpentadecyl hexanoate, 8-methylpentadecyl octanoate, 8-methylpentadecyl decanoate, and combinations thereof.

37. The method of claim 30 which has a viscosity ( $\text{Kv}_{100}$ ) from about 2 cSt to about 8 cSt at  $100^\circ \text{C}$ . as determined by 20 ASTM D445, a viscosity index (VI) from about 25 to about 150 as determined by ASTM D2270, a pour points from about  $-20^\circ \text{C}$ . to about  $-50^\circ \text{C}$ . as determined by ASTM D97, and a Noack volatility of no greater than 25 percent as 25 determined by ASTM D5800.

38. The method of claim 30 wherein the lubricating oil further comprises one or more of a viscosity improver, antioxidant, detergent, dispersant, pour point depressant, corrosion inhibitor, metal deactivator, seal compatibility 30 additive, anti-foam agent, inhibitor, and anti-rust additive.

\* \* \* \* \*